# EUROPEAN PATENT SPECIFICATION

(11) **EP 4 038 236 B1**
(45) Date of publication and mention of the grant of the patent: **30.10.2024**
(21) Application number: 20790167.9
(22) Date of filing: 30.09.2020
(51) Int. Cl.: D21H 19/38, B65D 65/42, D21H 21/54, D21H 27/10

(54) **RE-PULPABLE THERMALLY INSULATED PAPER PRODUCTS AND METHODS OF MAKING AND USING THE SAME**
WIEDERAUFLÖSBARE, WÄRMEISOLIERTE PAPIERPRODUKTE UND VERFAHREN ZU DEREN HERSTELLUNG UND VERWENDUNG
PRODUITS EN PAPIER ISOLANT THERMIQUEMENT RECYCLABLE ET MÉTHODES DE FABRICATION ET D'UTILISATION

(30) Priority: 01.10.2019 WO PCT/US2019/054121; 01.10.2019 US 201916590224; 01.04.2020 US 202016837129
(43) Date of publication of application: 10.08.2022
(73) Proprietor: OUTLIER SOLUTIONS, LLC, Chicago, IL 60622 (US)
(72) Inventor: FLYNN, Nigel, J., Flowery Branch, GA 30542 (US); LEIGH, Taylor, Kopacka, Alpharetta, GA 30005 (US); LYE, Jason, Atlanta, GA 30316 (US); SAY, Terence, Edwin, Powder Springs, GA 30127 (US)
(74) Representative: Weickmann & Weickmann PartmbB
(86) International application number: PCT/US2020/053421
(87) International publication number: WO 2021/067367

(56) References cited:
- WO-A2-2004/046463
- US-A- 5 155 138
- US-B1- 6 265 040
- US-B1- 6 740 373

## Description

### FIELD OF THE INVENTION

The present invention relates generally to repulpable insulated paper products. The present invention further relates to methods of using insulated paper products.

### BACKGROUND OF THE INVENTION

Food sold in fast food restaurants is often wrapped in a low basis weight paper product. The wrapping paper is often treated with a coating to provide wet strength, such as a silicone, or a fluorocarbon, or a wax, and further is often laminated to a thin aluminum foil. The aluminum foil serves several purposes. First, aluminum has a low thermal emissivity, and so the foil layer provides thermal insulation. Second, the foil adds some resiliency to the paper when subjected to hot moisture and lipids, such as vegetable and animal fats, dairy products etc.

While cheap to produce, manufacture, and effective at insulating, such laminated foil paper products also have many disadvantages. Aluminum foil (1) is persistent in the environment as it does not decompose, contributing to long term landfills, (2) is frequently litter that is unsightly and may cause obstruction in the guts of smaller animals when ingested, (3) is not recyclable or repulpable, causing problems if accidentally introduced into a repulping mill, (4) does not burn if the material is incinerated and (5) has been linked to certain neurodegenerative diseases in humans when ingested.

For similar reasons, some paper beverage cups are also difficult to recycle. They are coated with a low molecular weight polyethylene, which causes problems when introduced into the pulp.

What is needed is a highly thermally insulating paper structure that provides one or more of the following benefits: (1) is non-toxic and safe for use with food, (2) is thin and can be supplied to restaurants in roll or sheet format, (3) insulates hot food from cooling, (4) is recyclable by municipal recycling services without separation or segregation from other papers in the waste stream, (5) is biodegradable or biodestructable and therefore ephemeral when released into the environment (6) is able to maintain integrity with condensation formation after wrapping hot food, and (7) is resistant to the penetration of oils and fats.

### SUMMARY OF THE INVENTION

The present invention is directed to insulated paper products as defined in claims 1-13 that (1) insulate food positioned therein and/or surrounded thereby, (2) are biodegradable or biodestructable, recyclable, repulpable, and (3) can be printed and decorated, and (4) are food contact safe. The disclosed insulated paper products utilize a coating that acts in a similar manner to a laminated aluminum foil. Insulating materials included within the coating are coated onto a variety of paper products.

In another embodiment, the present invention is directed to a repulpable storage container comprising the insulated paper product of the present invention as defined in claim 14.

The present document further describes methods of making insulated paper products. A method of making an insulating wrapping paper product may comprise: forming a paper sheet comprising one or more layers on a fourdrinier wire, then coating the formed paper layer with a coating with a low thermal conductivity and/or a low thermal emissivity onto the paper layer. A method of making an insulating wrapping paper product may further comprise coating the formed paper layer with a moisture barrier and/or a grease resistant layer at the size press, and then coating a thin layer of a coating with a low thermal conductivity and/or a low thermal emissivity.

For example, a method of making an insulating wrapping paper product may comprise: forming a paper sheet comprising one or more layers, then coating the formed paper layer with a moisture barrier and/or a grease resistant layer on one side, and then coating a thin layer of a coating with a low thermal conductivity and/or a low thermal emissivity on the opposite side.

In another example, a method of making an insulating wrapping paper product may comprise: forming a paper sheet comprising one or more layers, then coating the formed paper layer with a moisture barrier and/or a grease resistant layer on one side, and then coating a thin layer of a coating with a low thermal conductivity and/or a low thermal emissivity on the same side.

The present invention is even further directed to methods of using insulated paper products as defined in claim 15. The method of using an insulated paper product comprises: insulating an object (e.g., food, medicine, pharmaceuticals, ice, flowers, etc.) via any one of the herein-described insulated paper products.

These and other features and advantages of the present invention will become apparent after a review of the following detailed description of the disclosed embodiments and the appended claims.

### BRIEF DESCRIPTION OF THE FIGURES

The present invention is further described with reference to the appended figure, wherein:
FIG. **1** depicts a perspective view of an exemplary paper product of the present invention;
FIGS. **2A-2C** depict exemplary cross-sectional views of the exemplary paper product shown in FIG. **1** as viewed along line **2-2** shown in FIG. **1****;**
FIG. **3** depicts a perspective view of another exemplary paper product of the present invention;
FIGS. **4A-4C** depict side views of exemplary paper products of the present invention;
FIG. **5** depicts a perspective view of another exemplary paper product of the present invention (also referred to herein as "an integral paper product");
FIGS. **6A-6D** depict exemplary cross-sectional views of the exemplary paper product shown in FIG. **5** as viewed along line **6-6** shown in FIG. **5****;**
FIGS. **7A-7C** depict an exemplary process flow in an exemplary papermaking process suitable for use in forming the exemplary paper products of the present invention;
FIG. **8** depicts a side view of another paper product forming process step suitable for forming an exemplary paper product of the present invention;
FIGS. **9A-9C** depict exemplary storage containers comprising any one of the exemplary insulated paper products of the present invention;
FIG. **9D** depicts an exemplary cross-sectional view of the wall structure of the exemplary hot beverage cup shown in FIG. **9C****;**
FIGS. **10-13A** depict additional exemplary storage containers comprising any one of the exemplary insulated paper products of the present invention;
FIG. **13B** depicts a close-up cross-sectional view of the wall structure of the exemplary shipping container shown in FIG. **13A****;**
FIG. **14** depicts an exemplary cross-sectional view of a wall structure of an exemplary shipping container;
FIGS. **15-17** depict views of another apparatus that may be used to determine the relative emissivity of paper samples and/or insulating materials;
FIG. **18** depicts a view of another apparatus that may be used to determine the relative emissivity of paper samples and/or insulating materials;
FIG. **19A** and **19B** depict views of an apparatus that may be used to determine the rate of heat transfer of paper samples and/or insulating materials with FIG. **19A** depicts a cut-away view of modifications to an expanded polystyrene cooler including dimensions, as well as positioning of the window through the cooler wall. FIG. **19B** depicts a cross sectional view of the test apparatus;
FIG. **20** depicts a corrugated structure of the present invention with one side coated; and
FIG. **21** depicts single faced corrugate paper hot beverage cup sleeves including the net and cross section.

### DETAILED DESCRIPTION OF THE INVENTION

The present invention is directed to insulated paper products as defined in claims 1-13 comprising fibers **11** (e.g., wood pulp fibers **11**) and insulating material **12.** Although shown in all figures, each paper layer **10** comprises fibers **11** (e.g., wood pulp fibers **11**) with or without other paper layer additives including, but not limited to, an insulating material **12.** Some definitions of fibers, paper, and packaging, as well as product specification and fiber sources, are provided below.

As used herein, the term "paper" is used to identify a type of non-woven material in which fibers are randomly oriented in all directions. Fibers principally made from cellulose are poured as a slurry on a mesh screen. As the paper is formed, the fibers come into contact with each other, and physically bond with neighboring fibers via a variety of interactions, including hydrogen bonding. The fibers originally come from plants including trees, although synthetic and mineral fibers, or other types of fibers, may optionally be included. Often, the paper also contains recycled fiber. Wood may be sourced from direct harvesting of trees from forest land, or from lumber industry byproducts (such as sawdust).

Paper fibers may include the fibrous portions from many parts, including softwoods (such as those plants with needles instead of leaves, for example, loblolly pine) and hardwoods. Other plants that yield useful paper fibers include but are not limited to bamboo, sugar cane, wheat straw, reed grass, mischanthus grass, coconut fiber, hemp fiber, cotton fiber, jute, palm, reeds, and papyrus. Cellulose fibers in many plants are bound together with lignin.

In the case of virgin (non-recycled) fiber, much of the lignin is removed during the pulping process. Recycled paper may include fibers from corrugated, fiber board, writing paper, pressboard, card, newspaper, tissue paper, specialty papers, linerboard, containerboard, boxboard, PE-lined paperboard, carton material, cup stock, or foodboard.

When made from trees, the pulping process involves methods to separate the individual cellulosic fibers into a slurry, as well as remove some or all of the lignin. Pulping methods may include a) thermomechanical pulping, which involves the use of steam and sheer forces generated between a spinning and a stationary plate, b) chemical pulping, which uses strong chemicals to break down the pulp by dissolving the lignin, and/or c) the semi-chem process, which uses a combination of mechanical and chemical methods. Most often, fluted medium board (e.g., fluted medium board 23) is made using semi-chem process pulp and/or recycled paper fiber. Other types of pulp include solid bleached sulfate pulp, chipboard, and kraft.

Paper (and paper layer **10**), as used herein, may broadly include any material that includes 15% or more cellulose fibers (discussed further below). Other additives, including insulating material **12,** other particles/additives/components that impart grease resistant and/or water resistant, as well as other particles/additives/components to impart strength. Non-paper (and non-paper layer **30**) is anything containing less than 15% of cellulose fibers (discussed further below).

As used herein, the term insulating material, such as insulating material **12,** is used to describe inorganic or organic materials that provide some degree of insulation. The term insulating material, as in insulating material **12,** does not include air alone or any other gas alone, although air and/or another gas could be trapped within one or more inorganic or organic insulating material **12.**

Paper products **10/100'/60,** comprising fibers **11** (e.g., wood pulp fibers **11**) and insulating material **12,** can either be made flat (e.g., insulated paper products **100/100'**) using a screen to make flat materials, or alternatively be molded, vacuum formed, or thermoformed from a pulp suspension to form essentially three-dimensional (non-flat) objects (e.g., molded or otherwise formed containers **60** shown in FIGS. **9A-13B**). Such three-dimensional paper products include certain packaging, for instance, egg crates and egg cartons, packaging that protects the corners of products shipped in the mail, biodegradable compost containers, biodegradable plant pots, disposable urinals and bed pans used in hospitals, disposable cat little boxes, and the like. Additives, including insulating material **12,** may be included within and/or on the paper products **10/100'/60** to impart thermal insulation properties, strength under moist or wet conditions, impart water repellency or water proofing, impart grease absorption resistance, increase strength, improve the color, improve printability, or other aesthetic aspects.

Additives, including insulating material **12,** may be added to the paper pulp prior to casting on the paper wire or otherwise molding the pulp with additives into a product **10/100'/60.** Alternatively, additives, including insulating material **12,** may be added at the size press, or after the steam can dryers. Additives, including insulating material **12,** can also be added to a clay coating (e.g., coating **30**) often applied to liner board (e.g., liner board **21/22**) to make clay coated kraftback, or clay coated newsback.

According to the invention, the insulating material is present in a thermally insulating coating as defined in claim 1.

Paper packaging (e.g., containers **60** shown in FIGS. **9A-13B**), formed from the insulated paper products **100/100'/100"** of the present invention, may include a wide variety of formats, including: regular slotted container (RSC), overlap slotted container, full overlap slotted container, special center slotted container, Bag-in-Box, center special overlap slotted container, center special full-overlap slotted container, snap- or 1-2-3-bottom box with tuck top, snap- or 1-2-3-bottom box with RSC top, Full Bottom File Box, Hamper Style, Ft. Wayne Bottom or Anderson Lock Bottom, Bellows Style top and Bottom Container, Integral Divider Container, RSC with Internal Divider or Self Divider Box, Full-telescope Design-style Box, Full-telescope Half-slotted Box, Partial-Telescope Design-style Box, Partial-telescope half-slotted box, Design-Style Box with cover, Half-slotted Box with cover, Octagonal Double Cover Container, Double cover box, Interlocking Double-Cover box, double-thickness score-line box, one-piece folder, two-piece folder, three-piece folder, fiver panel folder, one piece folder with air cell/end buffers (used to protect e.g. books), wrap-around blank, tuck folder, one piece telescope, double-slide box, number 2 or 3 bliss box, recessed end box, self-erecting box, pre-glued auto bottom with RSC top flaps, four corner tray, self-erecting six-corner tray, flange box, Arthur lock bottom, valentine lock container, reverse valentine lock container.

Medium board used in the insulated paper products **100/100'/100"** of the present invention may be fluted with flutes of different dimensions. See, for example, exemplary fluted medium board **23** shown in FIGS. **6A-6D**). The Fiber Box Handbook defines flutes and flute dimensions as: A, B, C, E, F, G, K, N, as well as R/S/T/D. The liner and medium papers may also be tested and rated by different burst grade: 125-350 SW, 23-55 ECT, 200-600 DW, 42-82 ECT DW, 700-1300 TW, 67-112 ECT TW. The carton or box (e.g., box **61**) may then be folded into the following industry known styles: reverse tuck, snap lock, automatic bottom, straight tuck, tuck top snaplock bottom, tuck top automatic bottom, seal end, beers, mailing envelopes, folder, and simplex.

Generally, an insulated paper product may comprise a single paper layer with insulating material dispersed therein or coated thereon, or may comprise two or more paper layers in combination with insulating material, wherein the insulating material is within one or more of the paper layers of the insulated paper product and/or is present as a component within the insulated paper product (e.g., as a separate layer from the paper layers and/or as a filler within a layer or component of the insulated paper product). See, for example, exemplary insulated paper products **100/100'/100"** in FIGS. **1-6D****.** According to the invention, the insulating material is present in a thermally insulating coating as defined in claim 1.

The insulated paper products of the present invention may further comprise one or additional layers other than the one or more paper layers and layers of insulating material. Suitable additional layers may include, but are not limited to, a coating that provides reduced emissivity of the insulated paper product, a coating that provides a desired color and/or surface texture for the insulated paper product, and a coating that provide enhanced water-repellency (e.g., waterproofing properties) to the insulated paper product. See, for example, exemplary insulated paper products **100/100'/100"** in FIGS. **6A-6D****.**

In exemplary insulated paper product **100/100'/100"** shown in FIG. **6A****,** a corrugated cardboard structure **100/100'/100"** comprises two liner boards **21/22** bonded to a fluted medium board **23.** One (or both) of the liner boards **21/22** may be coated (e.g., clay coated) with coating layer **30** for aesthetics. The fluted medium **23** may have a range of flute dimensions, which are classified by the industry as A-flute through F-Flute. Each liner board **21/22** may be made from one ply of paper **10/100',** or it may comprise two or more plies **10/100'.** Other types of board that could be used in combination with the above-described insulated paper products **100/100'/100"** discussed above: pressboard - pressed fiber board; honeycomb board - e.g., two liner boards **21/22** with a honeycomb spacer in between.

In exemplary insulated paper product **100/100'/100"** shown in FIG. **6B****,** a corrugated cardboard structure **100/100'/100"** comprises two liner boards **21/22** bonded to a fluted medium board **23,** and demonstrates several opportunities for incorporation of insulating additives **12** into the structure of corrugated cardboard **100/100'/100".** First, insulating additives **12** have been added to the furnish of the fluted medium **23.** Second, the flutes have been further isolated from heat transfer via conduction by incorporating insulating additives **12** into the starch adhesive **40** that bonds each flute (e.g., of fluted medium **23**) to the liner boards **21/22.** Third, the liner board **21** is coated with insulating additives **12** via a coating **30.** Fourth, to slow radiative heat transfer, a low emissivity coating **30** is overcoated on the outside of the corrugated cardboard structure **100/100'/100"** (e.g., a box **61**). Such a coating **30** will reflect vs. absorb radiative heat and infra-red radiation.

In exemplary insulated paper product **100/100'/100"** shown in FIG. **6C****,** another corrugated cardboard structure **100/100'/100"** comprises two liner boards **21/22** bonded to a fluted medium board **23,** and again demonstrates several opportunities for incorporation of insulating additives **12** into the corrugated cardboard structure **100/100'/100".** First, insulating additives **12** have been added to the furnish of the fluted medium board **23,** however, in such a way that the insulating material **12** has preferentially segregated to one face (e.g., the upper face as shown) of the medium fluted board **23** over the other (e.g., the lower face as shown). Second, the flutes (of the medium fluted board **23**) have been further isolated from heat transfer via conduction by incorporating insulating additives **12** into the starch adhesive **40** that bonds each flute of the medium fluted board **23** to the liner boards **21/22.** Third, another coating **310** containing insulating additives **12** has been incorporated in the valleys **231** of the flutes. Fourth, one of the liner boards **21/22** contains insulating additives **12** distributed in a non-uniform manner (e.g., such as in first liner board **21** as shown). Fifth, to slow radiative heat transfer, a low emissivity coating **30** is overcoated on the outside faces of both liner boards **21/22.** Such a coating **30** will reflect vs. absorb radiative heat and infra-red radiation. Emissivity relates to both a surface's ability to absorb and radiate heat. Thus, a low emissivity coating will also show reduced heat loss through radiative cooling.

In exemplary insulated paper product **100/100'/100"** shown in FIG. **6D****,** another corrugated cardboard structure **100/100'/100"** comprises two liner boards **21/22** bonded to a fluted medium board **23,** and again demonstrates several opportunities for incorporation of insulating additives **12** into the insulated paper product **100/100'/100".** First, insulating additives **12** have been added to the furnish of the fluted medium board **23** in such a way that the insulating materials **12** are distributed evenly throughout the thickness of the one or more paper layers **10/100'.** Second, the flutes of the fluted medium board **23** have been further isolated from heat transfer via conduction by incorporating insulating additives **12** into the starch adhesive **40** that bonds each flute of the fluted medium board **23** to the liner boards **21/22.** Third, another coating **30** containing insulating additives **12** has been coated onto one of the liner board **21.** Fourth, the second liner board **22** contains insulating additives **12** distributed in a non-uniform manner. Fifth, to slow radiative heat transfer, a low emissivity coating **30** is overcoated on the outside faces of one of the liner boards **21.** Such a coating **30** will reflect vs. absorb radiative heat and infra-red radiation. It will also show reduced heat loss through radiative cooling because emissivity relates to both a surfaces ability to absorb and radiate heat.

In addition, any of the insulated paper products of the present invention described herein may be configured into a variety of shapes. For example, in some embodiments, the insulated paper product is in the form of an insulated cup or mug that may be used to house a hot beverage such as coffee. Such insulated paper products may be used instead of STYROFOAM^{®} cups, eliminating the disposal and environmental problems associated with STYROFOAM^{®} cups. In other embodiments, the insulated paper product is in the form of insulated packaging for temporary storage and transport of items such as food, medicines, etc. Such insulated paper products may be in the form of an insulated box, corrugated or not corrugated, as well as many other packaging items discussed herein. See, for example, exemplary insulated paper products **100/100'/100"** in FIGS. **9A-13B****.**

Regardless of configuration and/or shape, the insulated paper products **100/100'/100"** of the present invention provide a degree of insulation due to coating compositions that reduce heat transfer.

The present document further describes methods of making and using the herein disclosed and described coated insulated paper products. The insulated paper products may be made using papermaking equipment and techniques so as to produce one or more paper layers. As discussed herein, the methods of making the insulated paper products of the present invention involve the strategic placement of one or more insulating materials within a given insulated paper product and/or the strategic placement of one or more optional coatings on the insulated paper product so as to provide superior insulating properties, as well as other properties to the insulated paper product. Exemplary method steps and procedures for forming insulated paper products of the present invention are shown/described in FIGS. **7A-7C** and FIG. **8****.**

FIGS. **7A-7C** depict an exemplary process of forming paper sheets **10.** As shown in FIG. **7A****,** pulp (furnish) is pumped into a header box **204.** The fiber content of the furnish is approximately 1-2 wt% at this stage. A gate **205** allows furnish to flow out onto the moving forming wire (a fine mesh conveyor.) **206.** The forming wire **206** may be 75-100 feet long. Initially, water drains via gravity, however, further down, vacuum boxes **207** beneath the wire **206** assist water removal, increasing the fiber content to around 20-30 wt%.

As shown in FIG. **7B****,** the material (~20-30 wt% fiber) is then fed through one or more felt presses **208,** which "blot" the precursor paper (i.e., precursor to paper layer **10**), removing more water, and increasing the fiber content to around 45-50 wt%. If starch or another additive or coating is to be applied, then that may be done at the size press **209** prior to drying. Many different materials may be added at the size press **209** prior to the dryers, including starch, sizes, waxes, coatings to impart wet strength, materials to impart water resistance, and materials that impart grease proofing.

As shown in FIG. **7C****,** drying may be affected in a number of ways, including running over steam cans **210,** or entering a long hot air-drying tunnel (not shown). After passing through calendar rolls **211** and prior to winding, the paper **10** may be between 6 to 10% moisture content.

FIG. **8** depicts details of an exemplary linerboard **100** suitable for use in forming an insulated paper product **100/100'/100"** of the present invention or a component (e.g., a layer or outer linerboard) of an insulated paper product **100/100'/100"** of the present invention. As shown in FIG. **8****,** exemplary linerboard **100** comprises two sheets of paper **10** laminated to one another. Exemplary linerboard **100** further comprises a first clay coating **30** directly on an outer surface **13** of one of the paper layers **10,** and an outermost second white clay coating **30** so as to provide a printable surface/layer **38** for exemplary linerboard **100.** First clay coating **30** evens out the valleys and troughs of the rough paper **10,** leaving a smooth surface for additional coatings and for high-quality printing.

The methods of using the insulated paper products **10/100/100'/100"** of the present invention may comprise insulating food, medicines, etc. from hot or cold environments. In some embodiments, the method may simply comprise placing an item (e.g., food, medicines, etc.) within an insulated paper product **10/100/100'/100"** of the present invention (e.g., putting hot coffee in a cup of the present invention). In other embodiments, the method may comprise placing an item (e.g., food, medicines, etc.) within an insulated paper product **10/100/100'/100"** of the present invention (e.g., a bag or a box), and sealing the insulated paper product **10/100/100'/100"** for transport.

As discussed herein, methods of using the insulated paper products **10/100/100'/100"** of the present invention may involve insulating an item (e.g., food, medicines, etc.) from hot or cold environments, wherein the item (e.g., food, medicines, etc.) is placed or packaged within an insulated paper product **10/100/100'/100"** that has a conventional shape, such as a cup or box. In other words, the insulated paper products **10/100/100'/100"** of the present invention take the place or conventional items such as cups and boxes so as to provide one or more advantages as discussed above. As discussed herein, the insulated paper products **10/100/100'/100"** of the present invention may have a variety of shapes and configurations similar to many conventional items such as cups and boxes.

During use, the insulated paper products **10/100/100'/100"/60** of the present invention desirably provide/have one or more of the following features/properties in addition to providing insulating properties:
(1) Moisture and Grease Resistance: Desirably, the insulated paper products **10/100/100'/100"/60** of the present invention (e.g., a box **61**) can be placed into a freezer and then taken out and stacked at room temperature. Such a process usually leads to the insulated paper product **10/100/100'/100"/60** (e.g., a box **61**) "sweating" through condensation in the warm air condensing on the surface of the insulated paper product **10/100/100'/100"/60** (e.g., a box **61**). In this regard, it is advantageous for the insulated paper product **10/100/100'/100"/60** (e.g., a box **61**) to be resistant to moisture ingress. Multiple different additives can be used to reduce the propensity of the insulated paper product **10/100/100'/100"/60** (e.g., a box **61**) to absorb moisture and weaken when moist. For example, perlite **12** is more hydrophobic than paper fibers **11,** so the incorporation of perlite **12** into and/or onto a paper layer **10** renders the paper layer **10** less absorbent. Further, the adhesive **40** that bonds flutes to liner board (see, FIGS. **6A-6D**) can be made moisture resistant by adding a moisture resistant adhesive resin, such as Coragum SR available from Ingredion, Westchester IL. In addition, a hydrophobic treatment can be applied to the exterior of the insulated paper product **10/100/100'/100"/60** (e.g., a box **61**). Moreover, a chemical cross-linking agent or reactive resin (e.g. a methylol melamine) may be applied to the insulated paper product **10/100/100'/100"/60** (e.g., a box **61**), so that it is less sensitive to moisture. Lastly, paper fiber **11** may be treated with rosin, and then aluminum sulfate can be added to the furnish to impart hydrophobicity to the paper layer **10.** Alternatively, a wax may be added to paper layer **10** to impart hydrophobicity. Commercial examples of water-resistant coatings that may be applied onto paper layer **10** include, Epotal S440 (BASF) (i.e., a styrene acrylic based copolymer emulsion), Rhoplex P-376 (Dow) (i.e., a styrene acrylic copolymer emulsion binder), Diofan B204 (Solvay) (i.e., a poly(vinylidene chloride) (PVDC) latex), Barrier-Grip 9471A (IGI) (i.e., a blend including a styrene acrylic copolymer emulsion, a poly(ethylene) wax and clay), Daran SL143 (Owensboro) (i.e., a poly(vinylidene chloride) (PVDC) latex). Of particular interest are moisture barriers that are repulpable, including Barrier-Grip 9471A, Aquaban, EC404 (a repulpable moisture barrier) from International Group Inc., (Toronto Canada.) or EcoShield Barrier Coating from Cortec Packaging. These proprietary commercial materials may include moisture and gas barrier additives and treatments such as low-molecular weight resins, waxes including paraffin wax and natural waxes such as beeswax, linear fatty acid esters of fatty alcohols, branched esters for example esters of 15-hydroxypalmitic acid, fatty alcohol ethers, hydrocarbons in the range of about C₁₅ to C₅₀, hydrocarbon resins, particularly petroleum resins, styrene resins, cyclopentadiene resins, and terpene resins. Such additives can be used in effective amounts, which vary depending upon the properties required.
   While undesirable from an environmental and recycling perspective, a thin layer of low density polyethylene (PE) may also be coated onto paper layer **10,** fiberboard **21/22/23,** and card stock to impart oil and water resistance, as is common practice in the fast food and hot & cold beverage retail industry. Alternatively, the surface of the paper may be cross linked by applying reactive groups that react with hydroxyl groups present in cellulose. For examples, melamine formaldehyde resins, urea formaldehyde resins, methylol melamine, epichlorohydrin, trichlorotriazine, dichlorotriazine, chlorotriazine coupled with diazabicylco-[2,2,2]-octane which acts as a catalyst, compounds that can undergo Michael 1,4 addition in the presence of base, and a wide range of other bifunctional reactive compounds. In recent years, the paper industry has experienced increased pressure to seek alternatives to PE liners and linings for packaging, leading the chemical industry to innovate new coatings that impart grease and water resistance while being repulpable. US 2019/0077537 to Georgia Pacific Bleached Board LLC teaches the use of several different coatings to impart resistance to water and lipid fluids to paper without the use of PE film, including Epotal S440 (BASF), Rhoplex P-376 (Dow), Diofan B204 (Solvay), Barrier-Grip 9471A (IGI), and Daran SL143 (Owensboro). These coatings were combined to impart heat seal-ability as well as water proofing to paper beverage cups.
(2) Transient Aluminized Layer for Low Emissivity: Addition of a thin aluminized coating **30** onto the paper (e.g., paper layer **10** and/or insulated paper product **100/100'** and/or corrugated paper product **100"** and/or storage container **60**) and/or onto the perlite **12** to lower emissivity. Aluminum has a very low emissivity and may be applied to various materials through a process called sputtering, or by vapor deposition. In this process, aluminum atoms traverse a vacuum and condense onto the surface of another material (e.g., paper layer **10**). Many thermal blankets are made via a process like this. Perlite particles **12,** as well as other types of particles, may be coated partially or totally in aluminum via these types of process. Paper or paper fibers **11** may also be metallized by an aluminum coating by similar processes. Aluminum foil and metalized plastic films do not re-pulp and have to be removed from the OCC and later waste streams, so these materials are not preferred in some embodiments of the present invention.
   However, it is possible to incorporate a chelating agent in another layer of the packaging (e.g., box **61**), or for instance in the adhesive, or in one of the coatings. Such a chelating agent would function to remove the aluminum during a pulping process. Chelating agents may include oxalic acid and oxalate salts, EDTA (ethylene diamine tetraacetic acid) and its various salts, salicylate, sodium hexametaphosphate and other materials. In this way, the aluminum could be removed. Soluble aluminum salts are already used in papermaking for instance as a flocculant for fines, as well as in combination with rosin soap to impart water resistance.
(3) Repulpable/Recyclable/Biodestructable: A repulpable/recyclable/biodestructable thermally insulating coating, comprising one or more inorganic pigments, which have been found to reduce the transfer of radiant heat energy when coated onto paper. The inventors found that a coating that included certain pigments such as mica, bismuth oxychloride, bismuth oxychloride coated mica, sericite, zinc oxide, zinc sulfide, cadmium sulfide will reduce the rate of radiative heat transfer through the coated paper.
(4) Odor Control and Taint of Foodstuffs: A concern with packaging and shipping of foodstuffs is taint and odor. This may arise from the inherent smell of virgin or recycled card, or it could arise when one package containing a strongly odorous material is placed in contact or adjacent to a package containing a food, beverage, drug, or tobacco product. There may be several ways to mitigate odor and taint of foodstuffs by incorporating materials into the paper structure. For instance, transition metal ion modified silica nanoparticles such as those described in U.S. Patent No. 7,976,855 are able to efficiently capture malodorous chemicals such as mercaptans, carboxylic acids, amine and other odors. U.S. Patent No. 8,168,563 teaches that silica nanoparticles may be modified by reaction with terminal aminoalkylthrimethoxysilanes and then with copper II ions to further enhance the odor capturing capabilities. Molecular sieves may also be included to sequester low molecular weight odor forming molecules such as hydrogen sulfide and zeolites to sequester ammonia and amine odors. Activated carbon was also found to impart thermal insulation, and would also be anticipated to absorb multiple odors. Activated carbon tends to be acidic in nature, and so may be especially good at taking up basic and weakly basic odors such as ammonia and amine odors. More complex odors also have an affinity for activated carbon, including mercaptan, thiol, and aromatic odors. Cyclodextrins, such as β-cyclodextrin or γ-cyclodextrin and their derivatives may also be incorporated for their odor absorbing properties. One or more of these materials/features could be incorporated into any of the here-in described paper layer **10** and/or insulated paper product **100/100'** and/or corrugated paper product **100"** and/or storage container **60** to modify and/or minimize any odors present.
   Odor transmission from one package to another, or from one good to another may also be mitigated through the use of barrier materials. As one object of the present invention is repulpability of packaging, aluminum foil, PE or PET film, and other synthetic materials would not be consistent with some embodiments of the present invention. However, some materials that provide thermal insulation have a microscopic flake morphology, such as mica and coated mica, and these materials may be useful for effectively blocking the transport of low and high MW malodor causing materials from ingress into packages (e.g., comprising or formed from insulated paper product **10/100/100'/100"**) of the present invention.
(5) Fiber Blend. Recycling, and Strength: Short length fibers tend to come from refined hardwood, while longer fibers come from softwood. A good ratio of 75% softwood 25% hardwood balances the properties of the two types of fiber, optimizing tensile strength. Recently, hemp fibers have come under increasing attention as a paper additive. Hemp fibers are far longer than other pulp fibers, help increase strength due to increasing contact points and bonding, and so may be subjected to multiple recycling steps - far more than regular wood fibers. Hemp fibers, being much longer than softwood may be recycled around 40 times vs. 6 for other types of fiber. One or more of these materials/features could be incorporated into any of the here-in described insulated paper layer **10** and/or insulated paper product **100/100'** and/or corrugated paper product **100"** and/or storage container **60.**
   In order to increase the ability of wood fibers to bond more through surface interactions, additional processes may be used to further fibrillate the fibers. For instance, the fibers may be subjected to an extreme high-shear environment, such as a colloid mill. The high sheer environment of two plate spinning in contact fibrillates cellulose fiber aggregates, increasing bonding, as well as the propensity to retain filler solids. Other ways to fibrillate the fiber can include prolonged beating in a mechanical Hollander pulp beater such as disclosed in the U.S. Patent No. 1,883,051 or by high-sheer mixing, high-speed mixing, or media milling. Fibrillated cellulose may increase porosity of the paper and paper strength due to enhanced bonding area between fibers. Other ways to increase strength is by including nanocellulose into the paper formulation. One or more of these materials/features could be incorporated into any of the here-in described paper layer **10** and/or insulated paper product **100/100'** and/or corrugated paper product **100"** and/or storage container **60.**
(6) Water Resistance Repulpability: Rosin is often used as part of a two-part system to impart moisture resistance in paper (e.g., paper layer **10** and/or insulated paper product **100/100'** and/or corrugated paper product **100"** and/or storage container **60**). The second part is post addition of aluminum salt solutions - e.g. aluminum chloride or aluminum sulfate. The aluminum reacts with the rosin soap to make a hydrophobic coating, which may impact repulpability yield. However, including a chelating agent somewhere in another component of the paper product may remove the aluminum from the rosin, thereby increasing the repulpability yield. Other areas of the paper that could carry the chelating agent may include the starch adhesive, and internal layer - for instance, the fluted medium, or an inner layer of the composite. Vapor-Guard R5341B or Barrier Grip 9471A (The International Group Inc., Titusville PA) are also useful as barrier coatings that provide the paper with a degree of grease and water resistance, and are described along with other suitable materials in Georgia Pacific Patent Application Publication No. US2019/0077537.
(7) Binders: Binders are used in coatings to reduce pigment rub-off, ensure adhesion of the coating, and generally seal the coating or ink. Binders for water-based coatings may be solutions such as poly(vinyl alcohol) or ammonia neutralized poly(acrylic acid). Binders that are latex based are more common, as they have a lower viscosity and are easier to formulate with and handle. As defined in claim 1, the paper product of present invention comprises from about 50.0 wt% to about 0.1 wt% of a latex binder as defined under item (A) or (B). Latex binders in general are a stable emulsion or dispersion of polymer particles or droplets in water. For instance, natural rubber latex sourced from trees comprises non-crosslinked cis-poly(isoprene) in microscopic droplets dispersed in water, with protein acting as a surfactant to stabilize the latex emulsion. Man-made latex binders according to item (A) are polymers synthesized using emulsion polymerization including poly(vinyl acetate), poly(acrylonitrile), poly(acrylates), poly(methacrylates), poly(butadiene), poly(styrene), poly(acrylic acid), and various copolymers of these polymers. As the water evaporates, the dispersed polymer particles come closer together, until the spherical droplets begin to touch. At first, the spheres become distorted in shape as the get closer. If the glass transition temperature ("Tg") of the polymer is low enough, chain intermingling between the touching droplets will begin to join the droplets together, forming a continuous film. According to item (B), a latex binder comprises a polymer or co-polymer of one or more monomers selected from styrene, butadiene, acrylic acid, acrylate, methacrylate, and vinyl acetate.

Rovene VSR-50 is an acrylic latex binder with pH in the range of 8-9, and around 45% solids content. The polymer contained in Rovene VSR-50 has a Tg of around 12°C, and so a heat treatment is needed to coalesce the dried polymer particles to form a film.

Rovene 4100 (Mallard Creek Polymers, NC) is a carboxylated styrene-butadiene copolymer emulsion with a polymer Tg around -5°C, so no post-dry heating is required to form a film. The product contains around 50% solids, and the emulsion has a pH of around 6. Rovene 6106 is a styrene-acrylic copolymer emulsion with a high Tg (>100°C), and so a post-heat treatment is required. Rovene 6090 is modified vinyl acetate copolymer emulsion with a polymer Tg of 39°C. This binder has release properties, allowing adhesive materials to be peeled from the coating surface.

Tykote 6160 (Mallard Creek Polymers) is an approximately 50% solids pH 8.0-9.0 acrylic polymer emulsion, with a polymer Tg of 7°C. This binder is claimed to have flexibility combined with moisture vapor barrier properties.

The present invention is further described by the following additional embodiments, examples, and claims. It should be understood that any feature and/or component described herein may be present alone or in combination with any other feature and/or component or combination of features and/or components described herein to form the here-in described paper layer **10** and/or insulated paper product **100/100'** and/or corrugated paper product **100"** and/or storage container **60** of the present invention. Examples that are not in accordance with the appended claims are described for illustrative purposes only.

### Insulated Paper Products

A repulpable insulated paper product **100** as defined in claim 1 comprises: one or more paper layers **10;** and an insulating coating **30** on at least one outer surface **13/15** of said one or more paper layers **10,** said thermally insulating coating **30** comprising (i) from about 50.0 weight percent (wt%) to about 99.9 wt% of one or more insulating materials **12** comprising bismuth oxychloride, mica, bismuth oxychloride-coated mica, zinc oxide, aluminum-doped zinc oxide, zinc sulfide, cadmium sulfide, bismuth vanadate, gypsum, sericite, powdered silicon, silver-coated glass bubbles, aluminum oxide, hollow polymeric microsphere pigments, or any mixture or combination thereof, and (ii) from about 50.0 wt% to about 0.1 wt% of a binder comprising (A) a latex binder selected from polymers synthesized using emulsion polymerization including poly(vinyl acetate), poly(acrylonitrile), poly(acrylates), poly(methacrylates), poly(butadiene), poly(styrene), poly(acrylic acid), and various copolymers of these polymers; or (B) a latex binder comprising a polymer or co-polymer of one or more monomers selected from styrene, butadiene, acrylic acid, acrylate, methacrylate, and vinyl acetate. The coating forms a continuous coating that completely covers the at least one outer surface; reflects heat; and reduces transfer of heat through the repulpable insulated paper product As discussed herein, each paper layer **10** may further comprise one or more additives, the one or more additives including, but are not limited to, flocculants and retention aids such as high molecular weight poly(acrylamide), poly(ethylene imine), cationic quar gum, and other cationic polymers; additives to provide water resistance (e.g., wax, synthetic latexes and resins); or any combination thereof. In some embodiments, the insulating coating **30** comprises one or more insulating materials **12** comprising bismuth oxychloride, mica, zinc oxide, zinc sulfide, cadmium sulfide, bismuth vanadate, sericite, or any mixture or combination thereof. In some embodiments, the insulating coating **30** comprises one or more insulating materials **12** comprising bismuth oxychloride, mica, zinc oxide, or any mixture or combination thereof.

In the insulated paper product **100,** the one or more paper layers **10** may comprise a single paper layer **10.**

Alternatively, the one or more paper layers **10** may compriss two or more paper layers **10.**

The insulating coating **30** may comprise one or more insulating materials **12** comprising bismuth oxychloride, mica, zinc oxide, aluminum-doped zinc oxide, zinc sulfide, cadmium sulfide, bismuth vanadate, sericite, or any mixture or combination thereof.

In particular,the insulating coating **30** may comprise one or more insulating materials **12** comprising bismuth oxychloride, mica, zinc oxide, aluminum-doped zinc oxide, or any mixture or combination thereof.

The insulating coating **30** comprises from about 50.0 weight percent (wt%) to about 99.9 wt% of the one or more insulating materials **12** and from about 50.0 wt% to about 0.1 wt% of the binder. It should be understood that the insulating coating **30** may comprise (i) any value between about 50.0 wt% and 99.9 wt%, in increments of 0.1 wt%, e.g., 95.7 wt%, or any range of values between about 50.0 wt% and 99.9 wt%, in increments of 0.1 wt%, e.g., from about 90.2 wt% to 98.1 wt%, of the one or more insulating materials **12,** and (ii) any value between about 50.0 wt% and 0.1 wt%, in increments of 0.1 wt%, e.g., 2.4 wt%, or any range of values between about 50.0 wt% and 0.1 wt%, in increments of 0.1 wt%, e.g., from about 18.3 wt% to 0.2 wt%, of the binder. The binders are as defined in claim 1 under items (A) and (B).

The insulating coating **30** may comprise from about 90.0 wt% to about 99.9 wt% of the one or more insulating materials **12** and from about 10.0 wt% to about 0.1 wt% of the binder.

In particular, the insulating coating **30** may comprise from about 93.0 wt% to about 98.0 wt% of the one or more insulating materials **12** and from about 7.0 wt% to about 2.0 wt% of the binder. According to the invention, the binder comprises a latex binder (A) or (B). A binder of item (B) is a latex binder comprising a polymer or co-polymer of one or more monomers selected from styrene, butadiene, acrylic acid, acrylate, methacrylate, and vinyl acetate.

Each insulating coating **30** may independently comprise one or more coating layers **30** with each coating layer **30** comprising said insulating material **12** and said binder.

At least one insulating coating **30** may comprise two or more coating layers **30** with each coating layer **30** comprising said insulating material **12** and said binder.

In particular embodiments, said two or more coating layers **30** comprise (i) a first coating applied onto the one or more paper layers **10** and comprising zinc oxide, aluminum-doped zinc oxide, or any mixture or combination thereof, and (ii) a second coating applied onto the first coating and comprising bismuth oxychloride, bismuth oxychloride-coated mica, or any mixture or combination thereof.

The insulated paper product **100** of the invention may further comprise a treatment to impart water or grease resistance to the insulated paper product **100.**

The treatment may comprise adding one or more treatment additives to one or more of the one or more paper layers **10.**

The treatment may comprise adding one or more treatment additives to the insulating coating **30.** Further, the treatment may comprise adding a water or grease resistance layer comprising one or more treatment additives onto the insulated paper product **100.**

In particular, the insulating coating **30** may be applied over the water or grease resistance layer.

In particular embodiments, the water or grease resistance layer is applied onto an outer surface of the insulated paper product **100** opposite the insulating coating **30.**

The one or more treatment additives may comprise a wax emulsion, a latex binder, Epotal S440 (BASF) (i.e., a styrene acrylic based copolymer emulsion), Rhoplex P-376 (Dow) (i.e., a styrene acrylic copolymer emulsion binder), Diofan B204 (Solvay) (i.e., a poly(vinylidene chloride) (PVDC) latex), Barrier-Grip 9471A (IGI) (i.e., a blend including a styrene acrylic copolymer emulsion, a poly(ethylene) wax and clay), Daran SL143 (Owensboro) (i.e., a poly(vinylidene chloride) (PVDC) latex), or any combination thereof.

The one or more treatment additives may comprise a wax emulsion, a latex binder, Epotal S440 (BASF) (i.e., a styrene acrylic based copolymer emulsion), Rhoplex P-376 (Dow) (i.e., a styrene acrylic copolymer emulsion binder), Diofan B204 (Solvay) (i.e., a poly(vinylidene chloride) (PVDC) latex), Barrier-Grip 9471A (IGI) (i.e., a blend including a styrene acrylic copolymer emulsion, a poly(ethylene) wax and clay), Daran SL143 (Owensboro) (i.e., a poly(vinylidene chloride) (PVDC) latex), or any combination thereof.

According to a particular aspect of the invention, the insulated paper product **100** has an overall basis weight of less than about 200 grams per square meter (gsm). It should be understood that the insulated paper product **100** may have any overall basis weight between about 40.0 gsm and 200.0 gsm, in increments of 0.1 gsm, e.g., 97.6 gsm, or any range of values between about 40.0 gsm and 200.0 gsm, in increments of 0.1 gsm, e.g., from 40.1 gsm to 160.0 gsm.

In particular embodiments, the insulated paper product **100** has an overall basis weight ranging from about 50.0 gsm to about 100 gsm.

The insulated paper product **100** may comprise a void-containing insulated paper product **100".**

In particular embodiments, the void-containing insulated paper product **100"** comprises voids **19** within at least one paper layer **10,** the voids **19** being encapsulated by a material other than paper (e.g., a paper layer **10** containing hollow beads/particles (not shown)).

The void-containing insulated paper product **100"** may comprise voids **19** within at least one paper layer **10,** the voids **19** being encapsulated by paper (e.g., a paper layer **10** containing air pockets **19** therein, possibly formed via a molding process or a process in which a void-forming material is removed from the paper layer **10**). See, FIGS. **5-6D****.**

The void-containing insulated paper product **100"** may comprise a corrugated paper product **100".**

According to a particular aspect of the invention, the integral paper product **100'** comprises (i) a first linerboard layer **21** comprising one or more first paper layers **10/100/100',** (ii) a second linerboard layer **22** comprising one or more second paper layers **10/100/100',** and (iii) (a) a fluted paper layer **23** comprising one or more fluted paper layers **10/100/100'** or (b) a honeycomb layer (not shown) positioned between the first linerboard layer **21** and the second linerboard layer **22,** and (I) each of (i) said first linerboard layer **21,** (ii) said second linerboard layer **22,** and (iii) (a) said fluted paper layer **23** or (b) said honeycomb layer (not shown) may independently comprise insulating material **12** therein or thereon, and (II) said insulating coating **30** is present on (i) an outer surface of said first linerboard layer **21,** (ii) an outer surface of said second linerboard layer **22,** or (iii) both (i) and (ii). An insulated paper product **100** according to claim 9 comprises a corrugated integral paper product **100",** said corrugated integral paper product **100"** comprising: a first linerboard layer **21** comprising one or more first paper layers **10/100/100',** a second linerboard layer **22** comprising one or more second paper layers **10/100/100',** and (a) a fluted paper layer **23** comprising one or more fluted paper layers **10/100/100'** or (b) a honeycomb layer (not shown) positioned between the first linerboard layer **21** and the second linerboard layer **22,** wherein one or more of (i) said first linerboard layer **21,** (ii) said second linerboard layer **22,** and (iii) (a) said fluted paper layer **23** or (b) said honeycomb layer (not shown) each independently comprise optional insulating material **12** therein or thereon; and a smooth, heat-reflecting, thermally insulating coating **30** on (i) an outer surface of said first linerboard layer **21,** (ii) an outer surface of said second linerboard layer **22,** or (iii) both (i) and (ii). According to a particular embodiment of the invention, (a) said fluted paper layer **23** or (b) said honeycomb layer (not shown) provides pockets of air **19** between said first linerboard layer **21** and said second linerboard layer **22.**

Said pockets of air **19** may represent from about 20 to 80 volume percent of a total volume occupied by (a) said fluted paper layer **23** or (b) said honeycomb layer (not shown)(i.e., a total volume between innermost opposing surfaces **25/27** of said first linerboard layer **21** and said second linerboard layer **22**). See, for example, FIG. **6A****.**

The insulated paper product **100** of of the above embodiments may further comprise an adhesive **40** that bonds portions of (a) said fluted paper layer **23** or (b) said honeycomb layer (not shown) to portions of said first linerboard layer **21** and said second linerboard layer **22.** Suitable materials for adhesive **40** include, but are not limited to, starch adhesives, synthetic latex adhesives such as poly(vinyl acetate), natural rubber latex, modified starches, hydrocolloids such as hydroxypropylcellulose, carboxymethylcellulose, and other water-soluble polymers such as poly(vinyl alcohol). A cross-linking agent may also be added to the adhesive to avoid potential swelling of the adhesive and weakening of the bonds when wet. Flocculants and retention aids may also be included such as high molecular weight poly(acrylamide), poly(ethylene imine), cationic quar gum, and other cationic polymers. As discussed herein, in some embodiments, adhesive **40** is at least partially filled with one or more of the herein disclosed insulating materials **12.**

In a particular embodiment, said adhesive **40** has insulating material **12** dispersed therein.

Each of (i) said first linerboard layer **21,** (ii) said second linerboard layer **22,** and (iii) (a) said fluted paper layer **23** or (b) said honeycomb layer (not shown) may independently comprise the insulated paper product **100** described above.

Alternatively, each of (i) said first linerboard layer **21,** (ii) said second linerboard layer **22,** and (iii) (a) said fluted paper layer **23** or (b) said honeycomb layer (not shown) is substantially free of insulating material **12.**

Alternatively, the integral paper product **100'** may comprise said fluted paper layer **23.** Alternatively, the integral paper product **100'** comprises said honeycomb layer (not shown).

According to a particular aspect of the invention, the insulated paper product **100'** further comprises one or more additional non-paper layers **20/30.** As used herein, the term "non-paper layer" is used to describe a layer that contains less than 5.0 wt% paper pulp or cellulosic fiber, and typically contains 0 wt% to less than 4.0 wt% paper pulp or cellulosic fiber. Conversely, as used herein, the term "paper layer" (such as each paper layer **10**) is used to describe a layer that contains 5.0 wt% or more paper pulp or cellulosic fiber, and typically contains greater than 6.0 wt% up to 100 wt% paper pulp or cellulosic fiber (or any value between 6.0 wt% and 100 wt%, in increments of 0.1 wt%, e.g., 50.0 wt%, or any range of values between 6.0 wt% and 100 wt%, in increments of 0.1 wt%, e.g., from 40.1 wt% to 70.2 wt%).

The one or more additional non-paper layers **20/30** may comprise a gypsum layer, a clay-containing layer, a polymer coating, a pigment-containing layer, a fabric layer (e.g., a nonwoven, woven or knit fabric layer), a fiber-reinforcement layer (e.g., a layer of unidirectional fibers), a second layer of insulating material **12,** a metal film layer, a foam layer, or any combination thereof. One or more of the additional non-paper layers **20/30** may be added to the insulated paper product **100** in order to provide a desire property such as lower (or higher) emissivity, lower (or higher) thermal conductivity, enhanced water-repellency, an aesthetically pleasing color and/or texture, or any combination thereof.

The one or more additional non-paper layers **20/30** may comprise a gypsum layer (not shown).

The one or more additional non-paper layers **20/30** may comprise a clay-containing layer **30,** a coating **30** that provides a lower or higher emissivity of the insulated paper product **100,** a pigment-containing layer **30,** or any combination thereof. See, FIG. **6A****.**

The one or more non-paper layers **20/30** may comprise at least two non-paper layers **20/30.**

In a particular aspect of the invention, at least one paper layer **10** of the one or more non-paper layers **10** comprise a paper insulating material **12.**

In particular, the paper insulating material **12** may comprise perlite, perlite coated with copper ions, expanded perlite, perlite hollow microspheres (such as available from Richard Baker Harrison Ltd., UK, or CenoStar Corporation (US), or Sil-Cel^{®} microcellular aluminum silicate filler particles made by creating a structure of multicellular spherical bubbles comprising perlite, available from Silbrico (US), Sil-Cel^{®} microspheres are available in a range of particle sizes, and may be coated or uncoated, or Dicaperl HP-2000 perlite microspheres, as sold by Dicalite (US), or flaked or milled perlite (such as Dicaperl LD1006, cryogenic grades of perlite, Dicaperl HP-100, HP-200, and HP100-40 grades, also sold by Dicalite), porous volcanic materials (such as pumice), vermiculite (including MicroLite^{®} vermiculite dispersions, available from Dicalite), hollow expanded vermiculite, glass foams (such as Owens Corning), recycled glass foams (such as manufactured by GrowStone Inc.), cellular glass insulation materials, cenospheres (such as available from CenoStar Corp.), glass bubbles (such as available from 3M under the trade designations iM30K, iM16k, and K20, as well as Q-Cel glass), ceramic microspheres, plastic microspheres, and synthetic hollow microspheres (such as available from Kish Company Inc.), silica aerogels (such as those available from Aspen Aerogels, and those that may be incorporated into paints and coatings under the Enova^{®} and Lumira^{®} brand from Cabot), microporous polyolefin-based aerogels (such as disclosed in US Patent Application Publication No. 2016/0272777 to Aspen Aerogels Inc.), organic aerogels such as those disclosed in PCT WO 2019121242 to Henkel AG & Co. KGAA which comprise thiol-epoxy based aerogels, xerogels (i.e., collapsed aerogels), seagels (i.e., microfoams made from agar and alginates), foamed starch, foamed paper pulp, agar, foamed agar, alginates, foamed alginates, bismuth oxychloride, metalized ceramics, metalized fibers, cadmium yellow pigment (cadmium disulfide), or any combination thereof. Examples of commercially available insulating materials 12 include, but are not limited to, FOAMGLAS^{®} products commercially available from Owens Corning (Pittsburg PA); and Growstone products commercially available from Growstone, LLC, a subsidiary of Earthstone International Inc. (Santa Fe, NM). Recycled glass suitable for use as insulating materials **12** is typically crushed to a finely divided powder and mixed with a blowing agent, e.g., carbon or limestone. It is then passed into a furnace hot enough to begin to melt the glass. As the glass powder particles begin to fuse, the blowing agent gives off a gas or vapor, forming bubbles inside the glass. This generates a porous, mostly closed cell glass foam, with high thermal and sound insulation properties. Vermiculite may also be used as a suitable insulating material **12.** Vermiculite is a hydrous phyllosilicate mineral that undergoes significant expansion when heated. Exfoliation occurs when the mineral is heated sufficiently, and the effect is routinely produced in commercial furnaces. Vermiculite is formed by weathering or hydrothermal alteration of biotite or phlogopite.

In particular embodiments, the paper insulating material **12** comprises perlite (e.g., in the paper **10,** the adhesive **40,** the coating **30,** and/or the emissivity coating **30**), aerogel (e.g., in the paper **10** and/or the adhesive **40**), glass bubbles (e.g., in the adhesive **40** and/or the coating **30**), activated carbon (e.g., in the paper **10,** the adhesive **40,** the coating **30,** and/or the emissivity coating **30**), or any combination thereof.

According to a particular aspect of the invention, the insulating material **12** comprises particles having an average particle size of less than about 1000 microns (µm) (or any average particle size greater than about 1.0 µm to less than about 1000 µm, in increments of 1.0 µm, e.g., 25 µm, or any range of average particle size less than about 1000 µm, in increments of 1.0 µm, e.g., from about 50 µm to about 500 µm). For example, perlite particles typically have an average particle size ranging from about 5.0 to about 150 µm, aerogel particles typically have an average particle size ranging from about 10 to about 800 µm, and glass bubble particles typically have an average particle size ranging from about 10.0 to about 50 µm.

The insulating material **12** may comprise particles having a multi-modal particle size distribution.

According to a particular aspect of the invention, any paper layer **10** that contains insulating material **12** comprises from 4.0 weight percent (wt%) to 99.0 wt% fibers **11,** and from about 96.0 wt% to about 1.0 wt% insulating material **12,** based on a total weight of the paper layer **10.** It should be understood that a given paper layer **10** that contains insulating material **12** can have (a) any weight percent of fibers **11** between 4.0 wt% and 99.0 wt% (i.e., in increments of 0.1 wt%, e.g., 55.5 wt%, or any range of values between 4.0 wt% and 99.0 wt%, in increments of 0.1 wt%, e.g., from 35.6 wt% to 74.1 wt%).

Any paper layer **10** that contains insulating material **12** may comprise from 5.0 wt% to 75.0 wt% fibers **11,** and from about 95.0 wt% to about 25.0 wt% insulating material **12,** based on a total weight of the paper layer **10.**

According to a particular aspect of the invention, the insulating material **12** has a material density of less than 1.0 gram per cubic centimeter (g/cm³), more typically, less than 0.6 g/cm³. It should be understood that the insulating material **12** can have any material density less than 1.0 g/cm³ such as from greater than 0.01 g/cm³ to about 0.99 g/cm³ (or any value between 0.01 and 0.99, in increments of 0.01 g/cm³, e.g., 0.48 g/cm³, or any range of values between 0.01 and 0.99, in increments of 0.01 g/cm³, e.g., from 0.10 g/cm³ to 0.50 g/cm³).

According to a particular aspect of the invention, at least one layer **10** of said one or more paper layers **10** has a layer density of less than 1.0 g/cm³. It should be understood that the at least one layer **10** can have any layer density less than 1.0 g/cm³ such as from greater than 0.01 g/cm³ to about 0.99 g/cm³ (or any value between 0.01 and 0.99, in increments of 0.01 g/cm³, e.g., 0.78 g/cm³, or any range of values between 0.01 and 0.99, in increments of 0.01 g/cm³, e.g., from 0.20 g/cm³ to 0.60 g/cm³). It should be further understood that any number of layers **10** of said one or more paper layers **10** may have an independent layer density, each of which is less than 1.0 g/cm³ (or any value between 0.01 and 0.99, in increments of 0.01 g/cm³, e.g., 0.88 g/cm³, or any range of values between 0.01 and 0.99, in increments of 0.01 g/cm³, e.g., from 0.15 g/cm³ to 0.55 g/cm³).

According to a particular aspect of the invention, the insulated paper product **100** is molded to form a three-dimensional object (e.g., a cup **62** or container **60**).

A repulpable storage container **60** according to claim 14 comprises the insulated paper product **100** of any one of embodiments described above. See, FIGS. **9A-9C****.**

The storage container **60** may comprise a storage volume **66** at least partially surrounded by one or more container walls **68.**

The storage volume **66** can be completely surrounded by or surroundable (i.e., the storage container **60** can be configured to surround the storage volume **66**) by one or more container walls **68.**

The one or more container walls **68** can comprise the insulated paper product **100** of any one of the above embodiments.

The one or more container walls **68** may comprise a gypsum layer, a clay-containing layer, a polymer coating, a pigment-containing layer, a bismuth oxychloride-containing layer, a mica containing layer, an aerogel containing layer, a fabric layer (e.g., a nonwoven, woven or knit fabric layer), a fiber-reinforcement layer (e.g., a layer of unidirectional fibers), a layer of insulating material **12,** a metal film layer, a foam layer, a layer of air, a coating that lowers an emissivity of the one or more container walls (e.g., such as mica, bismuth oxychloride, zinc oxide, zinc sulfide, kaolin clay, or cadmium sulfide), a coating that lowers a thermal conductivity of the one or more container walls, a coating that enhances a water-repellency of the one or more container walls such as a wax, or a fluorocarbon, or a reactive cross-linking agent such as an epoxy or a urethane, or a silicone-based coating, or one or more coatings mentioned in U.S. Patent Application Publication No. 2019/077537, or any combination thereof.

The storage container **60** may comprise an insulating wrapper for a food item.

In particular embodiments, the container **60** comprises a cup **62,** a mug, a flask, or a thermos **62.** As shown in FIG. **9C****,** the storage container **60** may be a hot beverage cup **62,** which could replace both STYROFOAM^{®} cups, as well as lined paper cups along with the insulating paper ring currently provided to prevent burning fingers of the person holding the cup.

In other embodiments, the container **60** comprises a clam shell type box packaging **60** for hot food **80.** Such a container may be made via molding pulp using a vacuum forming machine. See, for example, FIG. **10****.**

In still further embodiments, the container **60** comprises a salad container **60** for chilled food **80.** See, for example, FIG. **11****.**

In other embodiments, the container **60** comprises a padded envelope **60.** See, for example, FIG. **12****.** In other embodiments, the container **60** comprises a shipping container **60.** See, for example, FIG. **13A****.** As shown in FIG. **13B****,** exemplary shipping container **60** comprises (i) multiple thinner paper layers **10,** each of which optionally includes insulating materials **12** incorporated therein, optionally with (ii) a non-uniform distribution of material particles **92** (which could be insulating material **12**), optionally (iii) air **90** or an insulative filler material between the layers **10,** and (iv) optionally additional coating(s) **30** on one or more of the paper layers **10.**

The shipping container **60** may comprise shipping container walls **69** that comprise a closed cell foam **30'.** See, for example, FIG. In this embodiment, the closed cell foam **30'** may be a biodegradable foam **30',** for instance a foamed starch such as GreenCell^{®} sold by KTM Industries Inc. Holt, MI, or a foamed alginate, or pectin, or gelatin, or agar material that has been foamed through one means or another, and optionally chemically cross-linked to a certain extent. As shown in FIG. **14****,** the shipping container **60** may include paper layers **10** that may optionally include insulating material **12,** and may also contain a thermal barrier coating **30.** The coating **30** could be designed to reduce radiative heat transfer, or it could be designed to reduce conductive heat transfer, or it could be designed to reduce both.

In the storage container **60** or the insulated paper product **100** described herein, the insulating coating **30** can be present on (i) an inner surface **63,** (ii) an outer surface **13/15,** or (iii) both (i) and (ii) of the storage container **60** or the insulated paper product **100,** the insulating coating **30** having a low thermal emissivity or thermal barrier property. As used herein, the phrase "a low thermal emissivity" refers to a thermal emissivity of less than 0.90, as measured using Thermal Emissivity Method #3 Recommended by Flir Systems Inc. (described in the "Example" section below). Suitable materials for use in a given "emissivity coating" include, but are not limited to, bismuth oxychloride, mica flakes, perlite, kaolin, and any combination thereof (e.g., mica flakes partially or completely coated with bismuth oxychloride).

The treatment may comprise a coating **20/30** on (i) an inner surface **63,** (ii) an outer surface **13/15,** or (iii) both (i) and (ii) of the storage container **60** or the insulated paper product **100,** the coating **30** comprising one or more materials that increase the water resistance of (i) the inner surface **63,** (ii) the outer surface **13/15,** or (iii) both (i) and (ii) of the storage container **60** or the insulated paper product **100.**

A storage container **60** or the insulated paper product **100** described herein may further comprise a coating **20/30** on (i) an inner surface **63,** (ii) an outer surface **13/15,** or (iii) both (i) and (ii) of the storage container **60** or the insulated paper product **100,** the coating **20/30** water-proofing (i) the inner surface **63,** (ii) the outer surface **13/15,** or (iii) both (i) and (ii) of the storage container **60** or the insulated paper product **100.** By "waterproofing," it is meant that the outer surface **13/15** of the storage container **60** or the insulated paper product **100** can be in contact with water for 24 hours and maintain its structural integrity.

### Methods of Making Insulated Paper Products (not within the scope of the invention)

A method of making the insulated paper product **100** described herein may comprise coating the one or more paper layers on at least one side with the insulating coating **30.**

Said method may further comprise at least one papermaking step to form the one or more paper layers.

Said method may further comprise a treatment step to impart water or grease resistance to the insulated paper product **100.**

The treatment may comprise adding one or more treatment additives to one or more of the one or more paper layers **10.**

The treatment may comprise adding one or more treatment additives to the insulating coating **30.** The treatment may comprise adding a water or grease resistance layer comprising one or more treatment additives onto the insulated paper product **100.**

The insulating coating **30** can be applied over the water or grease resistance layer **30.**

The water or grease resistance layer can be applied onto an outer surface of the insulated paper product **100** opposite the insulating coating **30.**

The one or more treatment additives may comprise a wax emulsion, a latex binder, Epotal S440 (BASF) (i.e., a styrene acrylic based dispersion), Rhoplex P-376 (Dow) (i.e., a styrene acrylic binder), Diofan B204 (Solvay) (i.e., a polyvinylidene chloride (PVDC) latex), Barrier-Grip 9471A (IGI) (i.e., a styrene acrylic/PE wax/clay blend), Daran SL143 (Owensboro) (i.e., a polyvinylidene chloride (PVDC) latex), or any combination thereof.

The one or more treatment additives may comprise a wax emulsion, a latex binder, Epotal S440 (BASF) (i.e., a styrene acrylic based copolymer emulsion), Rhoplex P-376 (Dow) (i.e., a styrene acrylic copolymer emulsion binder), Diofan B204 (Solvay) (i.e., a poly(vinylidene chloride) (PVDC) latex), Barrier-Grip 9471A (IGI) (i.e., a blend including a styrene acrylic copolymer emulsion, a poly(ethylene) wax and clay), Daran SL143 (Owensboro) (i.e., a poly(vinylidene chloride) (PVDC) latex), or any combination thereof.

Said method may further comprise incorporating one or more additives into at least one paper layer **10** within the one or more paper layers **10.** Suitable additives include, but are not limited to, one or more insulating materials **12,** copper ions, waxes, synthetic (e.g., polymeric or glass) fibers, silica, surface modified silica, transition metal surface modified silica, cyclodextrin, sodium bicarbonate, silicones to impart grease and water resistance, metalized ceramic particles, metalized fibers, cationic starches, cationic polymers, such as cationic guar gum, poly(ethylene imine) (e.g., poly(ethylene imine marketed as Polymin P and available from Aldrich Chemical), fillers, sizes, binders, clays including bentonite clay, kaolin clay, and other minerals, calcium carbonate, calcium sulfate, and other materials that may be added to paper products for different reasons, and any combinations thereof. The filler may make the paper more receptive to printing, for instance, or make the paper glossy. Many fillers have a density greater than 1.0 g/cm³. Flocculants and retention aids, may also be included such as high molecular weight poly(acrylamide), poly(ethylene imine), cationic quar gum, and other cationic polymers. Sizes and binders may also be added to help provide strength to papers, and can include starches, hydrocolloids, artificial and natural polymer latexes, such as RHOPLEX^{®} acrylic resins from Dow Chemical and ROVENE^{®} binders from Mallard Creek Polymers (Charlotte NC). Water soluble polymers, such as poly(vinyl alcohol), and poly(acrylic acid) may also be added to the paper. Sometimes, water resistance on the final box is required. Vapor-Guard R5341B or Barrier Grip 9471A (The International Group Inc., Titusville PA) are useful as barrier coatings that provide a given paper layer **10** with a degree of grease and/or water resistance. Said method may further comprise forming at least one fluted paper layer **10** within the one or more paper layers **10.** See, for example, FIGS. **6A-6D****.**

The above method may further comprise: applying at least one additional layer onto the insulated paper product **100.** The additional layer could be another layer **20** of insulating material **12,** a coating **20/30** (e.g., a coating **30** that increases or decreases an emissivity of a paper layer **10/100"** or an integrated product **100"**), a non-paper layer **30,** a layer of air **90,** or any combination thereof. See, for example, FIGS. **6A-6D** and **14.**

Said method may further comprise forming a storage container **60.**

The storage container **60** may comprises the storage container **60** described hereinabove.

Said method may further comprise forming at least one paper layer **10** within the one or more paper layers **10** using recycled insulated paper product **100** described hereinabove. For example, one method of making at least one paper layer **10** and a container **60** formed therefrom comprises forming a corrugated structure **100"** with at least one outer ply/liner **21/22** that contains fiber **11** and insulating material **12,** and a fluted median ply/liner **23** without insulating material **12,** comprising: suspending cellulose fibers **11** in water to make paper pulp **11;** forming a fibrous first layer **10** from the pulp **11;** suspending cellulose fibers **11** in water, adding voided materials (e.g., hollow insulating material **12**), optionally adding surface active agents, optionally adding a flocculent; forming this layer **10** on top of the first layer of pulp **10;** suspending cellulose fibers **11** in water to make paper pulp **11;** forming a fibrous top layer **10** on top of the second layer **10;** pressing and drying the resultant three-ply insulated paper sheet **100';** optionally coating at least one of the surfaces of the three-ply insulated paper sheet **100'** with a coating **30** selected from comprising aluminum, silver, mica, sericite, zinc oxide, zinc sulfide, cadmium sulfide, bismuth oxychloride, bismuth oxychloride coated mica, bismuth vanadate, gypsum, or combinations thereof; passing a paper sheet **10** through a corrugator to make a fluted layer **23** while adhering two insulated paper sheets **100'** as liner boards **21/22** to the fluted layer **23** to form corrugated board **100";** optionally adding an additional fluted layer **23** and another liner board **21**or **22** to make a double walled corrugated structure **100",** containing three insulated liner boards **21/22** and two fluted layers **23;** cutting the double walled corrugated structure **100"** into the form/shape of a box **60;** and allowing the off-cuts (e.g., scraps from the cutting step) to be sent back to the repulping mill mixed with off-cuts from non-insulating board. Another method of making at least one paper layer **10** and a container **60** formed therefrom comprises forming a corrugated structure **100"** with at least one outer ply/liner **21/22** that contains a paper layer **10** and an insulating material layer **20,** and a fluted median ply/liner **23** without insulating material **12,** comprising: suspending cellulose fibers **11** in water to make paper pulp **11,** and optionally adding a flocculant; forming a fibrous first layer **10** from pulp **11;** suspending voided materials (e.g., hollow insulating material **12**) in water, optionally adding surface active agents, and optionally adding a flocculent and/or a binder; forming this layer **20** on top of the first layer **10** of pulp **11,** through curtain coating, slot-die coating, rod coating, spray application, etc.; suspending cellulose fibers **11** in water to make paper pulp **11** optionally adding a flocculant; forming a fibrous top layer **10** on top of the second layer **20;** pressing and drying the resultant insulated paper sheet **100';** optionally coating at least one of the surfaces of the resultant insulated paper sheet **100'** with a coating **30** comprising aluminum, silver, mica, sericite, zinc oxide, zinc sulfide, cadmium sulfide, bismuth oxychloride, bismuth oxychloride coated mica, bismuth vanadate, gypsum, or combinations thereof; passing a paper sheet **10** through a corrugator to make a fluted layer **23** while adhering two insulated paper sheets **100'** as liner boards **21/22** to the fluted layer **23** to form corrugated board **100";** optionally adding an additional fluted layer **23** and another liner board **21**or **22** to make a double walled corrugated structure **100",** containing three insulated liner boards **21/22** and two fluted layers **23;** cutting the double walled corrugated structure **100"** into the form/shape of a box **60;** and allowing the off-cuts (e.g., scraps from the cutting step) to be sent back to the repulping mill mixed with off-cuts from non-insulating board. Yet another method of making at least one paper layer **10** and a container **60** formed therefrom comprises forming a corrugated structure **100"** with at least one outer ply/liner **21/22** that contains fiber **11** and insulating material **12,** and a fluted median ply/liner **23** that comprises insulating material **12,** comprising: suspending cellulose fibers **11** in water to make paper pulp **11;** forming a fibrous first layer **10** from the pulp **11;** suspending cellulose fibers **11** in water, adding voided materials (e.g., hollow insulating material **12**), optionally adding surface active agents, optionally adding a flocculent; forming this layer **10** on top of the first layer of pulp **10;** suspending cellulose fibers **11** in water to make paper pulp **11;** forming a fibrous top layer **10** on top of the second layer **10;** pressing and drying the resultant three-ply insulated paper sheet **100';** optionally coating at least one of the surfaces of the three-ply insulated paper sheet **100'** with a coating **30** selected from comprising aluminum, silver, mica, sericite, zinc oxide, zinc sulfide, cadmium sulfide, bismuth oxychloride, bismuth oxychloride coated mica, bismuth vanadate, gypsum, or combinations thereof; passing the resultant three-ply insulated paper sheet **100'** through a corrugator to make a fluted layer **23** while adhering two insulated paper sheets **100'** as liner boards **21/22** to the fluted layer **23** to form corrugated board **100";** optionally adding an additional fluted layer **23** and another liner board **21or 22** to make a double walled corrugated structure **100",** containing three insulated liner boards **21/22** and two fluted layers **23;** cutting the double walled corrugated structure **100"** into the form/shape of a box **60;** and allowing the off-cuts (e.g., scraps from the cutting step) to be sent back to the repulping mill mixed with off-cuts from non-insulating board. Yet another method of making at least one paper layer **10** and a container **60** formed therefrom comprises forming a corrugated structure **100"** with at least one outer ply/liner **21/22** that contains a paper layer **10** and an insulating material layer **20,** and a fluted median ply/liner **23** with an insulating layer **20,** comprising: suspending cellulose fibers **11** in water to make paper pulp **11,** and optionally adding a flocculant; forming a fibrous first layer **10** from pulp **11;** suspending voided materials (e.g., hollow insulating material **12**) in water, optionally adding surface active agents, and optionally adding a flocculent and/or a binder; forming this layer **20** on top of the first layer **10** of pulp **11,** through curtain coating, slot-die coating, rod coating, spray application, etc.; suspending cellulose fibers **11** in water to make paper pulp **11** optionally adding a flocculant; forming a fibrous top layer **10** on top of the second layer **20;** pressing and drying the resultant insulated paper sheet **100';** optionally coating at least one of the surfaces of the resultant insulated paper sheet **100'** with a coating **30** comprising aluminum, silver, mica, sericite, zinc oxide, zinc sulfide, cadmium sulfide, bismuth oxychloride, bismuth oxychloride coated mica, bismuth vanadate, gypsum, or combinations thereof; passing the insulated paper sheet **100'** through a corrugator to make a fluted layer **23** while adhering two insulated paper sheets **100'** as liner boards **21/22** to the fluted layer **23** to form corrugated board **100";** optionally adding an additional fluted layer **23** and another liner board **21** or **22** to make a double walled corrugated structure **100",** containing three insulated liner boards **21/22** and two fluted layers **23;** cutting the double walled corrugated structure **100"** into the form/shape of a box **60;** and allowing the off-cuts (e.g., scraps from the cutting step) to be sent back to the repulping mill mixed with off-cuts from non-insulating board.

Said method may further comprise a molding step so as to form a three-dimensional object from the insulated paper product **100.**

The molding step may comprise a pressure molding step, a thermoforming step, a vacuum forming step, or any combination thereof.

Each paper layer **10** that contains insulating material **12** may comprise from 15.0 wt% to 99.0 wt% fibers **11,** and from about 85.0 wt% to about 1.0 wt% insulating material **12,** based on a total weight of the paper layer **10.**

Each paper layer **10** that contains insulating material **12** may comprise from 15.0 wt% to 80.0 wt% fibers **11,** and from about 85.0 wt% to about 20.0 wt% insulating material **12,** based on a total weight of the paper layer **10.**

The insulating material **12** may have a material density of less than 1.0 g/cm³ (or any value between 0.01 g/cm³ and 0.99 g/cm³, in increments of 0.01 g/cm³, e.g., 0.48 g/cm³, or any range of values between 0.01 g/cm³ and 0.99 g/cm³, in increments of 0.01 g/cm³, e.g., from 0.10 g/cm³ to 0.50 g/cm³). At least one layer **10** of the one or more paper layers **10** may have a layer density of less than 1.0 g/cm³ (or any value between 0.01 g/cm³ and 0.99 g/cm³, in increments of 0.01 g/cm³, e.g., 0.78 g/cm³, or any range of values between 0.01 g/cm³ and 0.99 g/cm³, in increments of 0.01 g/cm³, e.g., from 0.20 g/cm³ to 0.75 g/cm³). It should be further understood that any number of layers **10** of the one or more paper layers **10** may have an independent layer density, each of which is less than 1.0 g/cm³ (or any value between 0.01 g/cm³ and 0.99 g/cm³, in increments of 0.01 g/cm³, e.g., 0.44 g/cm³, or any range of values between 0.01 g/cm³ and 0.99 g/cm³, in increments of 0.01 g/cm³, e.g., from 0.18 g/cm³ to 0.85 g/cm³).

The integral paper product **100** may have an integral paper product density of less than 1.0 g/cm³ (or any value between 0.01 g/cm³ and 0.99, g/cm³ in increments of 0.01 g/cm³, e.g., 0.77 g/cm³, or any range of values between 0.01 g/cm³ and 0.99 g/cm³, in increments of 0.01 g/cm³, e.g., from 0.18 g/cm³ to 0.53 g/cm³).

### Methods of Using Insulated Paper Products

A method of using the insulated paper product **100** or the storage container **60** of the invention as defined in claim 15 comprises: insulating an object via the repulpable insulated paper product **100** or the storage container **60,** wherein the object is a food item, a medicine, or any other item that is desirably kept at a cool temperature (e.g., a temperature below room temperature or a refrigerating temperature) or at an elevated temperature (e.g., a temperature above room temperature or a hot-out-of-the-oven temperature).

In particular embodiments, the object is a food item.
in the method of use, the insulated paper product **100** may comprise an insulating wrapper for a food item.

In particular embodiments, the method uses the storage container **60** and the storage container **60** comprises a box **61, a** container **62** for temporarily housing a liquid (not shown), a cup, a mug, a flask, or a thermos **62, a** clam shell **60** for hot food **80** (See, for example, FIG. **10**.), a salad container **60** for chilled food **80** (See, for example, FIG. **11**.), a padded envelope **60** (See, for example, FIG. **12**.), a shipping container **60** (See, for example, FIG. **13A**), a shipping container **60** comprising shipping container walls **69** that comprise a closed cell foam **30'** (See, for example, FIG. **14**), or any combination thereof. For example, in one method of use, the method comprises a method of maintaining an object at a controlled temperature comprising: heating or chilling an object (e.g., food, medicine, meat, fish, salad, vegetables, flowers, pharmaceuticals, biological specimens) to a predetermined temperature T; packaging the object inside any herein-described storage container **60.** The storage container **60** of dimensions 12" x 10" x 7" can be capable of keeping a combination of 900 g cooked pork (or simulant) and 1800 g of frozen water gel packs (conditioned to -20°C prior to placing into the container) below 0°C after 10 hours in an external temperature of 23°C.

The method of use may further comprise transporting the object within the insulated paper product **100** or the storage container **60.**

The method of use may further comprise shipping the object within the insulated paper product **100** or the storage container **60.** For example, in one method of use, the method comprises a method of shipping an object at a controlled temperature comprising: chilling an object (e.g., food, medicine, meat, fish, salad, vegetables, flowers, pharmaceuticals, biological specimens) to below a spoiling temperature of the object; packaging the chilled object inside any herein-described storage container **60,** along with frozen water gel packs, dry ice, etc.; closing the container; placing the storage container **60** into a vehicle (e.g., car, train, bus, airplane, etc.); transporting the package to a predetermined destination; removing the storage container **60** from the vehicle; and delivering the storage container **60** to either the front door of a residence, or to the loading dock of a distribution center, or the entrance of a restaurant, or the receiving department of a business, wherein the temperature inside the unopened storage container **60** remains below the food spoiling temperature for at least 24 hours.

The method of use may further comprise repulping the insulated paper product **100** and/or the storage container **60** after said insulating step, wherein at least 80% of the insulating filler is removed from the pulp during the repulping operation.

The method of use may further comprise incorporating any fibers **11** and/or insulating particles **12** from a repulped insulated paper product **100** and/or a repulped storage container **60** into a newly formed insulated paper product **100** and/or a newly formed storage container **60.**

In addition, it should be understood that although the above-described insulated paper products and methods are described as "comprising" one or more components or steps, the above-described insulated paper products and methods may "comprise," "consists of," or "consist essentially of" the above-described components or steps of the insulated paper products and methods. Consequently, where the present invention, or a portion thereof, has been described with an openended term such as "comprising," it should be readily understood that (unless otherwise stated) the description of the present invention, or the portion thereof, should also be interpreted to describe the present invention, or a portion thereof, using the terms "consisting essentially of" or "consisting of" or variations thereof as discussed below.

As used herein, the terms "comprises," "comprising," "includes," "including," "has," "having," "contains", "containing," "characterized by" or any other variation thereof, are intended to encompass a non-exclusive inclusion, subject to any limitation explicitly indicated otherwise, of the recited components. For example, an insulated paper product and/or method that "comprises" a list of elements (e.g., components, layers or steps) is not necessarily limited to only those elements (or components or steps), but may include other elements (or components or steps) not expressly listed or inherent to the insulated paper product and/or method.

As used herein, the transitional phrases "consists of" and "consisting of" exclude any element, step, or component not specified. For example, "consists of" or "consisting of" used in a claim would limit the claim to the components, materials or steps specifically recited in the claim except for impurities ordinarily associated therewith (i.e., impurities within a given component). When the phrase "consists of" or "consisting of" appears in a clause of the body of a claim, rather than immediately following the preamble, the phrase "consists of" or "consisting of" limits only the elements (or components or steps) set forth in that clause; other elements (or components) are not excluded from the claim as a whole.

As used herein, the transitional phrases "consists essentially of" and "consisting essentially of" are used to define an insulated paper product and and/or a method that includes materials, steps, features, components, or elements, in addition to those literally disclosed, provided that these additional materials, steps, features, components, or elements do not materially affect the basic and novel characteristic(s) of the claimed invention. The term "consisting essentially of" occupies a middle ground between "comprising" and "consisting of".

Further, it should be understood that the herein-described insulated paper products and/or methods may comprise, consist essentially of, or consist of any of the herein-described components, layers and features, as shown in the figures with or without any feature(s) not shown in the figures. In other words, in some embodiments, the insulated paper products of the present invention do not have any additional features other than those shown in the figures, and such additional features, not shown in the figures, are specifically excluded from the insulated paper products. In other embodiments, the insulated paper products of the present invention do have one or more additional features that are not shown in the figures.

The present invention is described above and further illustrated below by way of examples, which are not to be construed in any way as imposing limitations upon the scope of the invention defined by the appended claims.

### EXAMPLES

Insulated paper products similar to exemplary insulated paper products **100/100'/100"/60** shown and described in FIGS. **1-21** were prepared.

### Example 1. Preparation of Insulated Paper Products:

### Test Methods:

### % solids analysis:

A polystyrene disposable weigh boat was accurately weighed to 4 decimal places (tare mass). Approximately 1-2 gram of liquid was placed in the weigh boat, and promptly weighed to four decimal places (gross-wet mass.) Subtracting the tare from the gross-wet mass gives the net-wet mass. The weigh boat was carefully tilted and rocked from side to side, allowing the liquid to coat the bottom of the weigh boat evenly, then it was placed in a cupboard for 24-48 hours to evaporate at room temperature. The dry weigh boat was re-weighed to four decimal places (gross-dry mass). Subtracting the tare from the gross-dry mass gives the net-dry mass. $% solids = 100 * net-dry/net-wet$ pH:
All pH measurements were made using universal indicator paper, as supplied by Micro Essential Laboratories Inc. The color of the paper and the chart were compared under indoor fluorescent strip lighting.

### Thermal Emissivity Comparison Method #1 (via conduction):

A modified version of Leslie's cube was used to screen multiple materials rapidly. The equipment is depicted in FIG. **15.** FIG. **16** shows the view from directly above the hotplate **70,** viewing the sample **10** in visible light. FIG. **17** shows the thermal view using the Flir E40 thermal camera **74.**

One complication with this test is that it highly thermally insulating materials will skew the results, as the method relies upon conduction of heat from the back to reach the same temperature. So, if the flux of heat traveling through is reduced significantly, then the black painted area will be cooling faster (through radiation) than sample area, leading to a slightly misleading result. For this reason, we developed several other tests to screen materials for emissivity.

### Materials:

- Paperboard sample(s) **10**
- Rectangular corrugated strips, 1.5" x 3"
- Calipers
- Digital hot plate **70** that heats to at least 37°C (98.6°F) and with a heating surface **71** at least 113 mm in diameter
- IR Camera **74** & Image Analysis Software
- Timer
- Polished aluminum strip **76,** 0.75mm thick, 2" x 3"
- Matte black spray paint (Rust-oleum High Performance Wheel, matte black)
- 3M Spray Adhesive

### Assumptions:

This test method assumes constant heat flow, and no edge losses or other effects from convection or radiation-based heat transfer (all the heat flows through the sample).

### Method:

1. Set the IR camera **74** to have an emissivity value of 0.95, or similar.
2. Turn on the hot plate **70** and set the temperature to 37°C. Once the hot plate **70** has reached 37°C, sample testing can begin. The temperature can be checked by using the IR camera **74.**
3. Cut 1.5" x 3" cardboard strips. Spray them evenly with 3M aerosol adhesive.
4. Generously sprinkle the material **12** to be testing over the cardboard, then tap to remove the excess.
5. Mask one half of the cardboard with aluminum foil, then spray paint the unmasked half of the sample with the matte black paint. Allow to dry (~45 minutes).
6. Turn on the hot plate **70** and set the temperature to 37°C. Once the hot plate **70** has reached 37°C, sample testing can begin. The temperature can be checked by using the IR camera **74.**
7. When ready to test:
   - Place the corrugated sample on top of the hot plate, painted side up
   - Place the polished aluminum also on the hotplate as a control.
   - Start a timer for 2 minutes
8. At the end of two minutes, take an IR image of the top surface **75** of the sample. Remove the cover plate and paper sample.
9. Repeat steps 6 & 7 until all samples have been tested.

### Analysis:

Use the thermal images to compare whether the sample is more or less emissive than the shiny or black painted portions.

The portion of the sample painted black has a high emissivity (approx. 0.90), and thus shows up red and displays the correct temperature. The polished aluminum material has a low emissivity (approx. 0.03), and thus shows up blue and displays a lower temperature than the object actually is.

So, for this test, one should be able to say whether the emissivity of the test sample is higher, lower, or roughly equal to the emissivity of the black or silver samples.

### Thermal Emissivity Method # 2 (By Illumination with an Incandescent Light Bulb):

FIG. **18** shows the test apparatus used to quickly visually compare the thermal emissivity of materials directly from the way that they absorb and then re-emit heat radiated from a hot-filament light bulb **83.** Samples were mounted onto a shiny metal plate **82.** Half of the sample was sprayed with mat black paint, and half was left exposed. All paint and adhesives used were allowed to dry at room temperature for at least 40 minutes. The camera **74** was switched on, and the spotlight was shone onto the samples from a low angle, so that stray heat radiation reflected away from the thermal camera **74.** Immediately, black and high emissivity materials lit up in the thermal camera screen, as the absorbed heat and then re-emitted it back out in all directions - including towards the thermal camera **74.**

Materials with low emissivity were generally much darker in color, after illumination for a few seconds.

### Thermal Emissivity Method #3 Recommended by Flir Systems Inc.:

The following procedure was found it the Flir E40 manual, to give an actual emissivity number. Method # 3 is as follows:
   Step 1: Determine the reflected apparent temperature. This is needed to compensate for reflected ambient radiation sources, reflecting from your sample. Here are the steps:
      i) Scrunch up a sheet of aluminum foil into a ball, and then uncrumple it.
      ii) Attach this to a sheet of card of the same size.
      iii) Put the cardboard in front of the object to me measured, with the foil pointing towards the camera **74.**
      iv) Set the internal camera emissivity setting to 1.0.
      v) Record the apparent temperature of the aluminum foil
   Step 2: Measuring the thermal emissivity:
      vi) Adhere a strip of black electrical tape to the sample.
      vii) Warm the sample up to at least 20°C warmer than the ambient temperature.
      viii) With the camera **74** pointing to the tape, change the emissivity setting to 0.97 and use one of the on-screen temperature measurement selection tools to measure the temperature of the tape.
      ix) Move the temperature measurement tool to the sample surface without the tape. Now, change the internal emissivity setting until the measured temperature matches that of the insulating tape.
      x) Record the emissivity of the sample.

### Thermal Emissivity Test Method #4:

Thermal emissivity of certain samples was also tested by Thermophysical Properties Research Laboratory, Inc. of West Fayetteville IN using the following test methodology.

The Table Top Emissimetry apparatus measures total normal emissivity over a broad wavelength band. Thin, square samples, 0.5" on a side are mounted facing downward on an isothermal copper block heated by a resistance heater and surrounded by ceramic insulation. Five type-K thermocouples are mounted on the bottom face of the isothermal plate. Sample temperatures during emissivity measurements are inferred from the closest thermocouple. The samples are exposed to ambient air with convection losses minimized by the face-down orientation of the samples and the small gap to the detector head.

The IR detector is a broadband thermopile with a 1 mm diameter sensitive area and flat spectral response from 1 - 40 micrometers wavelength. The detector and radiation shield are water cooled and view the sample through a 3.56 mm aperture 5 mm from the sample surface. The detector is sensitive to radiation from an approximately 4.57 mm diameter spot on the sample. Stray radiation on the detector is minimized by a flat optical black coating on the inner surface of the shield and both faces of the aperture plate and by cooling the shield and aperture plates. The shield temperature is monitored by two type-K thermocouples embedded in the shield walls. Thermocouple and detector voltages are fed to an analog to digital module and attached to a personal computer. The emissivity *ε* is calculated by the equation: $ϵ = \frac{{ϵ}_{shutter} \left({T}_{shutter}^{4}-{T}_{shield}^{4}\right) + S {ϵ}_{blkbody} \left({T}_{blkbody}^{4}-{T}_{shield}^{4}\right)}{\left(1+S\right) \left({T}_{Sample}^{4}-{T}_{Sensor}^{4}\right)}$ where: $S = \frac{\left({V}_{Sensor}-{V}_{shutter}\right)}{\left({V}_{blkbody}-{V}_{sensor}\right)}$ and V is the detector voltage, T is the temperature measured in Kelvin. The subscripts are as follows:
Tₛₕᵤₜₜₑᵣ is the temperature of the shutter.
T_{shield} is the temperature of the infrared detector when the shutter is in place.
Tₛₑₙₛₒᵣ is the temperature of the infrared detector during measurements.
T_{blackbody} is the temperature of the standard blackbody used to calculate the unknown values.
Tₛₐₘₚₗₑ is the temperature of the sample using the thermocouple nearest the sample.
Vₛₕᵤₜₜₑᵣ is the voltage from the infrared detector when the shutter is in place.
V_{blackbody} is the voltage from the two black body readings taken.
Vₛₑₙₛₒᵣ is the voltage of the infrared detector from each sample.
*εₛₕᵤₜₜₑᵣ* is the emissivity of the shutter at the temperature when read (*ε* = 0.09)
*ε_{blkbody}* is the emissivity of the blackbody standard (*ε* = 0.95)
*ε* is the emissivity of sample.

In operation, power to the heater is adjusted by a computer controlled Eurotherm temperature controller to achieve a desired plate temperature and the system is allowed to stabilize. The detector is aligned with the sample to be viewed and its output voltage recorded. All samples on the isothermal plate are maintained in a constant radiation and convective heat transfer environment as the X-Y table is moved by the extended insulation block surrounding the detector head. Measurement of an oxidized copper reference standard with *ε* = 0.96±0.01 and a closed aperture measurement are made before and after each sample suite at each temperature. Total hemispherical emissivity is estimated from total normal/total hemispherical relationships developed for metals and insulators. The current temperature range covered is from room temperature to around 150 °C.

### Expanded Polystyrene Cooler Window Test Method #5

This test was devised to measure the amount of heat flowing through a given sample, as if it were placed in direct sunlight on a hot day. While a steady-state test would be ideal, the inventors sought methods to make rapid assessments of thermal properties for further research. While not wishing to be limited by theory, this test combines both emissivity (absorption of radiative heat) and conduction to give a measure of the amount of heat passing through a given sample.

Approximately 5 US gallons of Atlanta city water was placed into a 6-gallon bucket and sealed with a lid to equilibrate to room temperature for at least 24 hours. Expanded polystyrene coolers were purchased from Uline (Pleasant Prairie WI) (part number S21529) Inside dimensions: 8" x 6" x7", wall thickness 1.5", and outside dimensions 11" x 9" x 10". A 100mm diameter acrylic circular template was used to draw a circle on one of the 11" x 9" faces of the cooler. The circle was positioned 60mm from the top of the cooler, and 88mm from either side, as shown in FIG. **43A-43B.** The circle was carefully cut out using an electrically heated hot knife (e.g. RoMech Pro Hot Knife Kit 200W Styrofoam cutter, made in China).

Two-part liquid silicone compound was mixed and used to seal the inside of the insulated cooler by painting the inner surfaces. The silicone resin (for example, Diamond Driven Liquid Silicone Compound, available from Amazon.com, or Oomoo 30 Silicone Mold Making Rubber available from Amazon, corn, or Smooth-On Ecoflex 00-35 fast platinum cure silicone rubber compound kit, available from Smooth-On through Amazon.com, or RTV Silicone Rubber for Mold Making available from Specialty Resin & Chemical LLC, Dowagiac MI, or similar) was allowed to cure overnight. The following day, excess silicone resin was cut from the exterior of the cooler in the vicinity of the cut circular hole, to ensure bondability between the expanded polystyrene and the sample. Although silicone resins were used, it was also found that epoxy resins could alternately be used to waterproof seal coolers without destroying the expanded polystyrene structure.

Sample preparation: Coatings were made onto 35 lb per 1000 sq ft (35 MSQ or 170 gsm) kraft board using meyer rods and dried. Example board is available from Juvo Plus Inc. (Irwindale CA) in the form of "200 pack kraft laser and ink jet printer post cards 2 up per page" SKU LJ-WACHG-031218-11-1. This paper was selected as it proved to be a more consistent source of kraft fiberboard than obtaining samples of 35 lb MSQ liner board from various corrugated board manufacturers. In some tests, the kraft fiberboard was substituted with a sheet of paper containing fillers, or thermal insulation elements or other materials that the inventors wished to assess, such as metallized bubble wrap.

Aluminum foil (e.g. Glad^{®} Heavy Duty Aluminum Foil, distributed by Phoenix Industries Inc Denver CO, and available in grocery stores) was cut into sheets which were sprayed black on the dull side, using matt black spray paint (e.g. Rust-Oleum^{®} Painter's Touch 2X Ultracover Paint + Primer, Rust-Oleum Corporation, Vernon Hills IL) and allowed to dry. The acrylic 100mm diameter template was then used to mark and cut circular samples of coated kraft board. The back (kraft paper) sides of these were then sprayed with an adhesive such as 3M^{®} Super 77 ^{™} Multipurpose Adhesive, made by 3M Company (Minneapolis MN) and sold in many craft, office, and hardware stores. The discs were carefully bonded to the shiny side of the painted foil, and placed between paper sheets under several books (about 1 kg pressure) until dry, to maintain flatness of the sample. The foil sheet was trimmed so that approximately 0.5" to 1" of shiny foil remained surrounded each sample.

3M^{®} Marine Adhesive Sealant Fast Cure 4000 UV (part # 05280) was then used to carefully adhere the black surface of the foil-sample composite to the outside of the cooler, so that the sample was in line with the opening into the cooler. Other sealants could be used provided that they bond to both painted foil and expanded polystyrene, do not destroy expanded polystyrene by partially dissolving it, and that they form a waterproof seal. This was then allowed to cure overnight.

The cooler with the sample window was placed on the test rig built and illustrated in FIGS. **19A-19B****.** The test rig allows the repeatable location of the test window in front of the 110V 250W tungsten filament heat lamp such as those used in restaurants to keep prepared food hot prior to serving (e.g. Intertek 5000707, white incandescent tungsten heat lamp). The test rig shown in FIGS. **19A-19B** includes adjustment of angle of incidence and distance from the surface of the lamp to the center of the test material. 4,500 g of water that had been allowed to equilibrate to room temperature was weighed to the nearest gram (using a Philips^{®} Essence kitchen electronic top pan scale 1g increments to 5 kg capacity) and poured into the cooler. The stirrer blade was inserted through the lid, and a digital thermometer probe was also inserted through the lid. A strobe light was used to time the rotation of the stir blade to 600 rpm.

The water was stirred for several minutes until the temperature stabilized, at which time it was recorded. A timer was set for 15 minutes. The heat lamp was switched on, and the timer started simultaneously. The temperature of the water in the cooler was recorded every 15 minutes for one hour.

All tests were conducted in an air-conditioned temperature-controlled environment with an air temperature between 68°F and 71°F. Positive control sample was a kraft disk that also had a layer of aluminum foil laminated to it before adhering it to the shiny side of black painted foil, and a negative control consisted of an uncoated kraft disk mounted onto a similar foil sheet.

The temperature rise (DT) over one hour was used to determine the amount of energy (Joules) flowing through the coated kraft board per unit time (Watts) using the equation: $E \left(Joules\right) = 4.2 * DT * 4500$ where 4.2 is the specific heat capacity of water in J.K⁻¹.g⁻¹; and 4500 is the mass of the water present in the container.

Rate of energy transfer into the water Watts (ER) through the window is calculated by dividing by the number of seconds in one hour, *viz*.: $ER = E/3600 Watts$ As the surface area of the disc is known, then the energy flux Watts per square meter can also be calculated (W.m⁻²)

In some experiments, an infrared thermometer (Etekcity Lasergrip 1025D) was also used to measure the outside temperature of the disk, to give an approximation of the temperature difference over the thickness of the sample.

### % Ash Content:

These tests were carried out by SGS Integrated Paper Services Inc., Appleton WI according to TAPPI T 211 om-16 Ash in wood, pulp, paper and paperboard: combustion at 525°C. Approximately 10.0 g of paper was accurately weighed, and then ashed in a muffle furnace at 525°C. The remaining ash was then re-weighed to determine ash content.

### % Moisture:

These tests were carried out by SGS Integrated Paper Services Inc., Appleton WI according to TAPPI T 550 om-13 Determination of equilibrium moisture in pulp, paper and paperboard.

### Repulpability:

Repulpability was tested by SGS Integrated Paper Services Inc., Appleton WI according to the "Voluntary Standard for Repulping and Recycling Corrugated Fiberboard treated to Improve its Performance in the Presence of Water and Water Vapor Protocol of 2013", generated by the Fiber Box Association, headquartered in Elk Grove Village, IL, 60007. Repulpable means the test material that can undergo the operation of re-wetting and fiberizing for subsequent sheet formation, using the process defined in this standard. In the repulpability test, materials are weighed, pulped in a specific manner using laboratory equipment, run through a laboratory disintegrator, and then run through a screen. The amount of rejected material is compared to the material that could be reused as pulp to make board as a % by mass. Two figures are derived: The first is the acceptable recovery of the fiber based upon the mass of material first entered into the test, and the second is the percentage of the recovered fiber that is accepted, not rejected. These figures constitute the "% re-pulpability", and the fiber box association has determined that a pass for both measures of repulpability is >85%. Other parameters recorded are: a) material fouling the equipment during pulping or forming b) material that does not disintegrate and has to be removed (becomes part of the rejects)

### Coating Method:

A clip attached to a ¾" thick glass plate is used to hold a stack of photocopy paper and the sheet of paper to be coated. A strip of masking tape was placed along the top of the sheet to be coated, and a paper towel was left hanging off the end. A transfer pipette was used to make a line of coating on the masking tape. This prevented the coating from prematurely soaking into the paper board to be coated. Meyer rods (available from RD Specialties Inc.) were used to draw the coating down over the sheet. The coating was then dried under ambient conditions.

### Wetting Out and Stabilization:

Before materials can be included in a coating or into the fibrous matrix of paper, materials first have to be wetted out and dispersed. Some materials such as glass have high enough surface free energy that the wet out spontaneously - whereas materials such as perlite and aerogel require surfactants to lower the surface free energy of the water enough to wet out the material.

Surfactants may be non-ionic, cationic, or anionic. They may be high molecular weight polymers or copolymers, or they may be low molecular weight, and able to reach newly created interfaces rapidly. Surfactants for aqueous systems may be characterized by their HLB value. HLB stands for Hydrophilic-Lipophilic Balance, and is a measure of the capability of the particular surfactant to wet out various surfaces of differing surface free energy. Very hydrophobic materials have a low surface free energy, so a matching surfactant should also have a low HLB value. More hydrophilic surfaces - those with multiple polar groups perhaps, require surfactants with higher HLB values.

Microspersion EZ manufactured by Micropowders Inc. of Tarrytown NJ is a non-ionic low molecular weight surfactant with a low HLB. Dawn^{®} liquid dish soap, manufactured by the Procter & Gamble Co (Cincinnati OH) is an example of a low molecular weight anionic surfactant. E-Sperse 100 (from Ethos, Greenville SC), Triton BG-10 (Dow) Glucopon 425 N (BASF) and Glucopon 215 UP (BASF) are additional materials that can wet out certain hydrophobic materials. The Surfynol ^{®} range available from Evonik are ethoxylated acetylenic diols of fairly low molecular weight. They are non-ionic, and low foaming due to the molecular interactions of the acetylenic moiety with the water surface. Surfynol 104, 440, 420 are representative examples.

Higher molecular weight materials are useful for stabilizing dispersions of various materials in water. Polymers may be anionic, cationic, or non-ionic - or have a mixture of characteristics. Polymeric dispersants, also known as "grid aids" are often co-polymeric in nature, for instance some of the Joncryl resins from BASF are believed to be methacrylic acid - styrene - butylmethacrylate copolymers, containing anionic ionizable groups. Zetasperse 3100, Zetasperse 3800, TegoDispers 752W, and TegoDispers 755W are also higher molecular weight dispersing agents with a net negative formal charge when ionized available from Evonik. Disperbyk 190, as well as other Disperbyk products available from BYK Chemie (Wallingford CT) are also polymeric / copolymeric materials that help stabilize dispersions through a) increasing particle surface negative charge (electrokinetic stabilization), and b) by allowing steric stabilization by dint of segments of polymer dissolving into the continuous medium.

### Low Emissivity Insulative Clay Coatings:

Many corrugated cardboard boxes and fiberboard packages are coated with a clay coating. This coating provides a smooth flat ink-receptive surface that allows high quality printing, it covers the brown color of unbleached pulp with white, and gives the packaging a higher quality feel. Often the coating is applied in two layers. The first layer is kaolin clay based, whitened by calcium carbonate. This layer helps smooth the surface by filling in low spots. The second layer also contains titanium dioxide and calcium carbonate. The formulations of clay coatings vary. Usually, they contain kaolin clay, along with a film forming binder, such as an acrylic latex, or sometimes a cornstarch. A polymeric dispersant is usually included to stabilize the clay coating, and a viscosity control agent is usually also included, such as carboxymethyl cellulose, or an hydrophobically associated alkali swellable polymer (HASE polymer.) Calcium carbonate is also usually included, along with titanium dioxide pigment for whitening. The clay coating offers another opportunity to incorporate insulative elements that reduce conduction and radiative heat transfer.

### Emissivity Screening Results of Materials - Conductivity Method #1:

Powdered materials were sampled and tested to observe emissivity differences through a thermal camera. The emissivity of the powder surface and the powder surface sprayed with black paint were compared. NVD = no visible difference.

| Material | Comment after 2 minutes of heating |
|---|---|
| Aerogel IC 3120 powder | Possible lower emissivity |
| Perlite P-32 75 micron (cenosphere) | NVD |
| Thermacel powder | Possible lower emissivity |
| Hi Refractive Index glass beads 60µ | Possible lower emissivity |
| Hi Refr. Index glass beads 35 µ-45µ | NVD |
| Hi Refr. Index glass beads 180 µ-600µ | NVD |
| Titanium dioxide powder | Lower |
| Zinc oxide powder | NVD |
| Yellow oxide pigment (iron oxide) | NVD |
| Bismuth oxychloride powder | Lower |
| Party pink mica powder | NVD |
| Super pearly white mica powder | NVD |
| Snowflake sparkle mica powder | Lower |
| Queens purple mica powder | NVD |
| Diatomaceous Earth powder | NVD |
| Mica Sheet | Lower |
| Kaolin Clay powder | NVD |
| Silicon powder | Lower |
| Kaolin Coating - 42-02 | Lower (slight) |
| Diatomaceous earth coating 43-01 | Lower (slight) |

These powder sample data gave us several ideas for follow up tests. Curiously, some of the materials gave different results if they are first formulated into a coating (e.g. kaolin and diatomaceous earth). In other cases, low thermal conductivity may have skewed some readings.

### Emissivity Screening Results of Materials - Illumination Method #2:

Both powdered materials, as well as materials incorporated into coatings coated onto fiberboard were sampled and tested to observe emissivity differences through a thermal camera. The emissivity of the powder surface/coating surface and regular Cardboard were compared when illuminated by an incandescent tungsten spot light. NVD = no visible difference in emissivity vs. cardboard. Coating formulas follow below. NT = not tested

| Material | Comment 4 seconds of illumination |
|---|---|
| Aerogel IC 3120 powder | NVD |
| Silicon powder | NVD |
| Snowflake Sparkle Mica | Lower |
| Pewter Silver mica | NVD |
| Hi RI glass beads 60µ Al coated | NVD |
| Hi Refr. Index glass beads 35 µ -45µ | Slightly lower |
| Thermacels | NVD |
| Titanium dioxide | Lower |
| Zinc oxide | Lower |
| Mica Sheet | Much Lower |
| Bismuth oxychloride powder | Much Lower |
| Perlite P-32 (75 µ) | NVD |
| 30-03, Meyer #130 (25% glass bubbles) | Slightly lower |
| 22-02, Meyer#130, (24% Aerogel in starch) | Lower |
| 19-01, Meyer#130, (37% Perlite in starch) | Much Lower |
| 19-01, Meyer #40, (37% Perlite in starch) | Lower |
| Kaolin Powder | Slightly Lower |
| Kaolin Coating - 42-02 Meyer #40 | Much Lower |
| Diatomaceous Earth powder | Lower |
| Diatomaceous earth coating 43-01 | NVD |
| Aerogel Coating 38-02 (-50% aerogel) | Much Lower |
| Bismuth Vanadate | Much Lower |
| BiLite 20 | Much Lower |
| Gypsum | Lower |
| Sericite Pigment | Lower |
| Aluminum Oxide Powder | Lower |

These data gave us additional ideas to pursue insulating against thermal radiative emission and absorption, in addition to insulating against thermal conduction.

### Additional Material Sources:

Glass beads, including high refractive index glass, and retroreflective hemi-spherically mirrored glass beads - Cole Safety Products,
Glass microbubbles - 3M specialty materials, iM30K
Bismuth oxychloride - Making Cosmetics Inc (Redmond WA). This is a pearlescent pigment, commonly used in cosmetics and packaging to impart a pearl effect. Other sources include BASF, as Biju Ultra UFC and Pearl Glo.
BiLite 20 powder - BiOCl coated onto mica flakes (BASF)
Bismuth Vanadate - Dominion Colour, Ontario
Titanium Dioxide - Brambleberry (Bellingham, WA)
Zinc Oxide - Brambleberry (Bellingham, WA), and Sky Organics
Snowflake Sparkle Mica - Brambleberry (Bellingham, WA)
Super Pearly White Mica - Brambleberry (Bellingham, WA)
Pewter Mica - Brambleberry (Bellingham, WA)
Party Pink Mica - Brambleberry (Bellingham, WA)
Queens Purple Mica - Brambleberry (Bellingham, WA)
Yellow iron oxide powder - Brambleberry (Bellingham, WA)
Thermacels - HyTech Thermal Solutions, Melbourne FL. This material is an additive that is advertised to be mixed into paint in order to increase the paint's insulating properties.

Rhoplex VSR-50 is an acrylic low VOC film forming binder emulsion in water. Commonly used in architectural coatings. Originally sold by Rohm & Haas, now available from Dow Chemical.

Sericite comprised sericite mica surface treated with magnesium myristate or Sericite White sparkle luxury mica colorant pigment powder by H&B Oils Center Co.

Supertherm paint, from Eagle Specialty Coatings, British Columbia, Canada

### Coatings to test for Emissivity on Fiberboard or Card

| Formulation ID | Materials | Quantity / g |
|---|---|---|
| JL 48-01 | CaCO₃ | 50.00 |
| | Water | 50.00 |
| | 10% Rhoplex VSR-50 in water | 20.00 |
| JL 48-02 | Kaolin Clay | 50.00 |
| | Water | 70.00 |
| | 10% Rhoplex VSR-50 | 20.00 |
| JL 48-03 | Bismuth Oxychloride | 20.13 |
| | water | 33.55 |
| | 10% Rhoplex VSR-50 in water | 8.05 |
| HT 50-01 | Eagle Specialized Coating | |

### Low Emissivity Coatings on Fiberboard - Cooler Window Tests

Based upon the rapid testing using Emissivity tests 1 & 2, several materials were selected for further investigation. In preparation for printing, fiberboard is often coated with a clay coating, which smooths the surface and gives it a white color. A simple clay coat formulation was generated: Kaolin Clay Coating 127-01:

| Material | Quantity (g) | |
|---|---|---|
| Water | 130 | |
| Tego Dispers 755W | 4.86 | Evonik |
| Rovene 6400 | 52.89 | Mallard Creek Polymers |
| Hydrite SB60 | 157.8 | Imerys |

### Low Emissivity Coating Formulations by % composition

| % | TS110 | 137-02 | TS111 | TS112 | TS113 | 137-06 | 127-02 | 137-04 | 137-05 | 136-01 |
|---|---|---|---|---|---|---|---|---|---|---|
| Water | 62.5 | 68.15 | 64.28 | 65.51 | 65.51 | 65.51 | 65.51 | 17.5 | 30.48 | 65.55 |
| T-755W | 8.18 | 2.5 | 5.01 | 5.10 | 5.10 | 5.1 | 5.1 | | | 5.1 |
| R-6090 | 2.75 | | | | | | | | | |
| R-4100 | | 2.85 | 2.71 | 2.85 | 2.85 | 2.85 | 2.85 | 2.85 | 2.85 | 2.85 |
| HPMC | | | 1.96 | | | | | | | |
| BiOCl | 26.56 | | | | | | | | | |
| BiLite | | 26.5 | | | | | | | | |
| ZnO | | | 26.04 | | | | | | | |
| ZnS | | | | 26.54 | | | | | | |
| MgO | | | | | 26.54 | | | | | |
| TiOz | | | | | | 26.5 | | | | |
| Al-ZnO | | | | | | | 26.54 | | | |
| TH1000 | | | | | | | | 80 | | |
| TH500EF | | | | | | | | | 66.67 | |
| Ag-Glass bubbles | | | | | | | | | | 26.5 |

| | | | | | | | | | | |
|---|---|---|---|---|---|---|---|---|---|---|
| ZnO - Sky Organics T-755W - a slightly anionic, polymeric high performance wetting and dispersing additive commercially available under tradename TEGO^{®} Dispers 755 W (Evonik (Allenton, Pennsylvania)) R-6090 - all acrylic emulsion commercially available under tradename Rovene^{®} 6090 (Mallard Creek Polymers (Charlotte, NC)) R-4100 denotes Rovene 4100 (Mallard Creek Polymers, NC) is a carboxylated styrene-butadiene copolymer emulsion with a polymer Tg around -5°C, so no post-dry heating is required to form a film. The product contains around 50% solids, and the emulsion has a pH of around 6. R-6090 denotes Rovene 6090 (Mallard Creek Polymers, NC) is a modified vinylacetate copolymer emulsion with a polymer Tg of 39°C. This binder has release properties, allowing adhesive materials to be peeled from the coating surface. HPMC - 3% aq solution of hydroxypropyl methyl cellulose. BiOCl - Bismuth oxychloride, sold as Pearl Glo (BASF) Al-ZnO - Aluminum-doped zinc oxide particles, AZO 100, 20-40 nm particle size, available from Oocap Inc. Las Crusas NM. TH500 EF is Ropaque^{™} TH500EF from Dow Chemical hollow polymeric microsphere pigment of approximate size 0.4 micron diameter, and 30% solids. TH1000 is Ropaque^{™} TH1000 from Dow Chemical hollow polymeric microsphere pigment of approximate size 1 micron diameter, and 26.5% solids Silver (Ag) -coated glass bubbles, available from CoSpheric LLC. Conductive silver metal coated hollow glass microspheres 5-30 microns, density 0.75g/cm³, product ID: M-18-Ag-0.75 | | | | | | | | | | |

Kaolin clay coating 127-01 was coated onto 170 gsm (35 lbs/1000 sq ft) kraft laser & inkjet printer post cards, available from Juvo Plus Inc Irwinsdale CA, using a # 5 Meyer rod and dried in a hot air oven at 250°F for 5 mins. Various coatings were selected and coated onto the board, drying the coatings between each application. A representative area was selected, and tested on the test rig illustrated in FIG. **19A-19B****.** The distance to the lamp was set to 4.5", 4500 grams of water were weighed into the cooler, and the stirrer rotation was set to 600 rpm. The water temperature rise over 1 hour of lamp exposure was recorded.

| Exp: | Al foil | none | 1 clay | 2 clay | 3 clay | BiOCl | BiLite | MgO |
|---|---|---|---|---|---|---|---|---|
| Base: | Kraft | Kraft | Kraft | Kraft | Kraft | Kraft | Kraft | Kraft |
| Coat 1 | Al foil | - | 127-01 | 127-01 | 127-01 | 127-01 | 127-01 | 127-01 |
| Coat 2 | - | - | - | 127-01 | 127-01 | TS110 | 137-02 | TS113 |
| Coat 3 | - | - | - | - | 127-01 | - | - | - |
| Temp Rise/°C | 1.3 | 4.1 | 3.7 | 3.5 | 3.5 | 3.4 | 3.1 | 3.5 |
| W.m⁻² | 87 | 274 | 247 | 234 | 234 | 227 | 207 | 234 |

| | | | | | | | | |
|---|---|---|---|---|---|---|---|---|
| Al foil: Aluminum foil (Reynolds heavy duty kitchen foil) was mounted dull face down to Juvo kraft paper using 3M spray adhesive. | | | | | | | | |

| Exp: | ZnO | ZnS | TiOz | Al.ZnO | AgGls* | TH1000 | TH500 EF | TiO2 on Foil |
|---|---|---|---|---|---|---|---|---|
| Base: | Kraft | Kraft | Kraft | Kraft | Kraft | Kraft | Kraft | Kraft |
| Coat 1 | 127-01 | 127-01 | 127-01 | 127-01 | 127-01 | 127-01 | 127-01 | Foil |
| Coat 2 | TS111 | TS112 | 137-06 | 127-02 | 136-01 | 137-05 | 137-04 | 137-06 |
| Coat 3 | - | - | - | - | - | - | - | - |
| Temp Rise/°C | 3.2 | 3.3 | 3.5 | 5.1 | 3.1 | 3.7 | 3.3 | 2.9 |
| W.m⁻² | 214 | 221 | 234 | 341 | 207 | 247 | 221 | 194 |

| | | | | | | | | |
|---|---|---|---|---|---|---|---|---|
| * Ag-coated glass bubbles, available from CoSpheric LLC. Conductive silver metal coated hollow glass microspheres 5-30 microns, density 0.75g/cm³, product ID: M-18-Ag-0.75 | | | | | | | | |

| Exp: | BiLite | ZnO | BiOCl | | ZnO/ BiLite | BiLite / ZnO |
|---|---|---|---|---|---|---|
| Base: | Kraft | Kraft | Kraft | | Kraft | Kraft |
| Coat 1 | 127-01 | 127-01 | 127-01 | | 127-02 | 127-02 |
| Coat 2 | 127-01 | 127-01 | 127-01 | | TS111 | 137-02 |
| Coat 3 | 137-02 | TS111 | TS110 | | 137-02 | TS111 |
| Temp Rise/°C | 3.2 | 3.1 | 3.3 | | 3 | 3.1 |
| W.m⁻² | 214 | 207 | 221 | | 201 | 207 |

These data suggest that we can reduce the amount of energy absorbed by a box, or emitted from the inside surfaces of a box using coatings, by around 30%. While aluminum foil, as well as aluminized bubble wrap are very effective, they can cause problems if introduced into the repulping stream, and in any case are challenging to recycle. Not only could many of these coatings be applied to the interior and or exterior of the box, but could also be used as separate sheets of packaging, as illustrated as the loose sheets in FIG. **13A-13B****.**

### Results of Emissivity Testing by Test Method #4:

| Exp: | Contrl | 1 clay | 2 clay | 3 clay | TiO₂ | ZnS | AgGls* | ZnO |
|---|---|---|---|---|---|---|---|---|
| Base: | Kraft | Kraft | Kraft | Kraft | Kraft | Kraft | Kraft | Kraft |
| Coat 1 | - | 127-01 | 127-01 | 127-01 | 127-01 | 127-01 | 127-01 | 127-01 |
| Coat 2 | - | - | 127-01 | 127-01 | 137-06 | TS112 | 136-01 | TS111 |
| Coat 3 | - | - | - | 127-01 | - | - | - | - |
| *ε* @ 23º*C* | 0.900 | 0.859 | 0.883 | | 0.885 | 0.869 | 0.519 | 0.888 |
| *ε* @ 30º*C* | 0.909 | 0.866 | 0.894 | | 0.895 | 0.873 | 0.530 | 0.918 |
| *ε* @ 40º*C* | 0.915 | 0.866 | 0.894 | | 0.904 | 0.874 | 0.536 | 0.933 |

| | | | | | | | | |
|---|---|---|---|---|---|---|---|---|
| * Ag-coated glass bubbles, available from CoSpheric LLC. Conductive silver metal coated hollow glass microspheres 5-30 microns, density 0.75g/cm³, product ID: M-18-Ag-0.75 | | | | | | | | |

| Exp: | BiLite | BiLite | ZnO | BiOCl | | ZnO / BiLite | BiLite / ZnO |
|---|---|---|---|---|---|---|---|
| Base: | Kraft | Kraft | Kraft | Kraft | | Kraft | Kraft |
| Coat 1 | 127-01 | 127-01 | 127-01 | 127-01 | | 127-02 | 127-02 |
| Coat 2 | 137-02 | 127-01 | 127-01 | 127-01 | | TS111 | 137-02 |
| Coat 3 | - | 137-02 | TS111 | TS110 | | 137-02 | TS111 |
| *ε* @ 23º*C* | 0.856 | 0.873 | 0.885 | 0.861 | | 0.848 | 0.868 |
| *ε* @ 30º*C* | 0.873 | 0.875 | 0.897 | 0.876 | | 0.860 | 0.877 |
| *ε* @ 40º*C* | 0.882 | 0.871 | 0.902 | 0.881 | | 0.856 | 0.881 |

### Discussion of Emissivity vs. Heat Transfer Results

The inventors were surprised by the results of their own emissivity tests methods 1 and 2, as well as the emissivity results provided by the outside laboratory (Thermal Emissivity Test Method #4). Several coatings have been discovered by the inventors that apparently reduce the transfer of radiant heat energy from an incandescent light bulb (as a proxy to the full-sun illumination of a delivered package) through sheets of paper. The inventors were surprised to find that the emissivity results from the third-party laboratory did not correlate with the heat transfer through the materials measured by the cooler window tests. Clearly, the inventors may have discovered several coatings with non-obvious and unexpected thermal properties.

| Sample | Emissivity at 23°C | Thermal Conduction / W.m⁻² |
|---|---|---|
| Clay+ZnO+BiLite | 0.848 | 201 |
| Ag-coated glass | 0.519 | 207 |
| Clay+BiLite+ZnO | 0.868 | 207 |
| Clay+Clay+ZnO | 0.885 | 207 |
| Clay+BiLite | NT | 207 |
| Clay+Clay+BiLite | 0.861 | 214 |
| Clay+ZnO | 0.888 | 214 |
| Clay+ZnS | 0.869 | 221 |
| Clay+Clay+BiOCl | 0.861 | 221 |
| Clay+TiO₂ | 0.885 | 234 |
| Clay+Clay | 0.883 | 234 |
| Clay | 0.859 | 237 |
| Kraft | 0.900 | 274 |

### Example 3. Sheets Containing Insulating Elements:

Approximately 5.35g portions of 35 lb liner board (International Paper) was shredded and repulped. Additional materials were added, along with surfactants if necessary for wetting. While not yet optimum formulations, we had found that we could make paper sheets containing insulating elements by adding surfactant, along with a cationic polysaccharide, such as cationic Guar Gum, available from Making Cosmetics Inc., or a cationic starch sizing, or a synthetic retention aid, such as Polymin P (BASF), also known as poly(ethylene imine), or a high molecular weight poly(acrylamide) available from various sources. Hydrophobically associating polymers may also be incorporated, such as N-alkyl poly(acrylamides.) We wished to understand the amount of retained insulation in the paper following drying.

The following formulations were made up and cast as paper, dried at room temperature and then sent for ash content and moisture content analysis:

| Formulation ID | Materials | Mass/g | Target % By mass | % Moisture paper | % Ash Paper |
|---|---|---|---|---|---|
| JL 24-02 Control | Water | 800.00 | | | |
| | Pulp | 5.35 | 0% | 8.4 % | 0.84 % |
| JL 23-01 | Water | 800.00 | | | |
| | Pulp | 5.35 | | | |
| | Microspersion EZ (neat) | 2.00 | | | |
| | Perlite P-50 (20 micron) | 1.78 | 25% | 6.2 % | 15.9 % |
| | Cationic Guar Gum | 0.80 | | | |
| JL 23-02 | Water | 800.00 | | | |
| | Pulp | 5.35 | | | |
| | Microspersion EZ (neat) | 2.00 | | | |
| | Perlite P-50 (20 micron) | 5.35 | 50% | 7.2 % | 28.5 % |
| | Cationic Guar Gum | 0.80 | | | |
| JL 24-01 | Water | 800.00 | | | |
| | Pulp | 5.35 | | | |
| | Microspersion EZ (neat) | 2.00 | | | |
| | Perlite P-50 (20 micron) | 5.35 | 50% | 6.7 % | 22.9 % |
| | Cationic Guar Gum | 2.00 | | | |
| JL 25-02 | | 800.00 | | | |
| | Pulp | 5.35 | | | |
| | Microspersion EZ (neat) | 2.50 | | | |
| | Perlite P-50 (20 micron) | 1.78 | 25% | 8.0 % | 8.8 % |
| pH = 8-9 | Polymin P | 0.80 | | | |
| JL 26-01 | Water | 800.00 | | | |
| | Pulp | 5.35 | | | |
| | Microspersion EZ (neat) | 2.00 | | | |
| pH = 6.0 | Perlite P-50 (20 micron) | 5.35 | 50% | 7.3 % | 16.8 % |
| JL 32-01 | Water | 800.00 | | | |
| | Pulp | 5.35 | | | |
| | 3M Glass Bubbles | 1.78 | 25% | 7.5 % | 14.7 % |
| | 0.5% a.q. Cationic Guar Gum | 10.00 | | | |
| JL 32-02 | Water | 800.00 | | | |
| | Pulp | 5.35 | | | |
| | 3M Glass Bubbles iM30K | 5.35 | 50% | 6.8 % | 28.5 % |
| | 0.5% a.q. Cationic | 10.00 | | | |
| Guar Gum | | | | | |

A mass balance was performed to confirm that a portion of the perlite and a portion of the finer was lost during the drawing and pressing process.

### Repulpability Tests: Insulated Paper vs. Uline Insulated Cardboard Box

90 lb fiberboard was fed through a paper shredder. 5.35g was weighed and pulped in hot water as usual. The pulp was more dense and more difficult to disperse than the pulp from the 35 lb paper. Paper sheets were made using the following formulations:

| | | |
|---|---|---|
| JL 41-01 | water | 800.00 |
| | Pulp - 90# shredded paper | 12.50 |
| | iM30K glass bubbles | 12.50 |
| | 0.5% cationic guar gum solution | 25.00 |
| JL 41-02 | | |
| | water | 800.00 |
| | Pulp - 90# shredded paper | 12.50 |
| | Microspersion EZ (neat) | 1.60 |
| | Perlite P-50 | 12.50 |
| | 0.5% cationic guar gum solution | 25.00 |

As a control (JL 44-01), the existing method of shipping cold objects was also tested for repulpability. Corrugated cardboard from a BS121007 single walled 12" x 10" x 17" box sections were laminated to an insulated box liner, made from 3/16" cool-shield bubble & metallized film, available from Uline as model number S-15223. The materials were laminated using 3M aerosol spray adhesive.

| Designation | Summary | Yield based upon total fiber collected. (% accepts) Av. of 2 | Yield based upon original charge to the pulper (% accepts) Av. of 2 | Operational impact (Pass/Fail) |
|---|---|---|---|---|
| 44-01 | Control | 64.7 % | 56.4 % | Fail |
| 41-01 | 50% iM30K | 98 % | 70 % | Pass |
| 41-02 | 50% perlite P-50 | 93 % | 66.9 % | Pass |

These data illustrate the validity that the approach of incorporating insulating elements into the paper structure has the potential to produce a repulpable thermally insulating material for packaging.

### Example 4. Additional Sheets Made for Moisture, Ash Content and Repulpability:

35 lbs per 1000 sq. ft. single-ply sheets containing additives were made for additional repulpability tests, consistent with the Fiberboard Association voluntary standard for repulpability. Sheets FA, FD, FE, FF, FG were made using Grade 100 bleached pulp secondary fiber (supplied by Donco Recycling Solutions with offices in Chicago IL.) The target basis weight for each sheet was 35 lbs per 1000 square feet (MSQ). Taking sample FD as an example, to make 35 MSQ board with 50% additive, 17.5 lbs of dry pulp is mixed with 17.5 lbs of additive for every 1,000 square feet of paper. Once ash content and moisture were measured, the sheets were then run through the repulping test in duplicate:

### Sample Details, Moisture, and Ash Content:

| Sample Details | | | Test Results | | | |
|---|---|---|---|---|---|---|
| | | | Measured % Moisture Content | Based upon Dried Material | | |
| ID | Additive | % Additive | | % Fiber | % Ash | % additive retention |
| FA | (control) | 0 | 8.4 | 98.7 | 1.4 | N/A |
| FD | 20*µ* spherical perlite | 50 | 5.4 | 56.9 | 43.1 | 86.1 |
| FE | iM30k glass bubbles | 50 | 5.1 | 54.5 | 45.5 | 90.9 |
| FF | Dicalite LD 1006 | 50 | 5.0 | 52.6 | 47.4 | 94.7 |
| FG | 75*µ* spherical perlite | 50 | 6.2 | 62.1 | 37.9 | 75.7 |

### Repulpability test data:

| ID | Initial Charge / g | Repulped Mass / g | Total Repulped mass accepted / g | Total Repulped mass Rejected / g | Total Fines/ g |
|---|---|---|---|---|---|
| FA | 25.20 | 21.06 | 21.06 | 0.000 | 4.14 |
| FA | 21.60 | 17.62 | 17.62 | 0.000 | 3.98 |
| FD | 25.20 | 14.21 | 13.87 | 0.251 | 11.08 |
| FD | 25.10 | 14.81 | 14.80 | 0.008 | 10.29 |
| FE | 25.70 | 12.09 | 12.09 | 0.000 | 13.61 |
| FE | 25.40 | 12.74 | 12.74 | 0.000 | 12.66 |
| FF | 25.10 | 14.64 | 14.64 | 0.004 | 10.46 |
| FF | 25.60 | 15.98 | 15.24 | 0.036 | 10.32 |

### Repulpability Test Results Analysis - Taking Ash Content Into Account:

| ID | % Accepts based upon total fiber collected | % Accepts based upon initial charge | % accepts based on the amount of fiber present in the initial charge (additive ash excluded) | Deposition on equipment noted: |
|---|---|---|---|---|
| FA | 100.0 | 83.6 | 84.0 | No |
| FA | 100.0 | 81.6 | 82.1 | No |
| FD | 98.2 | 55.0 | 85.8 | No |
| FD | 99.9 | 59.0 | 89.6 | No |
| FE | 100.0 | 47.0 | 75.2 | No |
| FE | 100.0 | 50.2 | 80.0 | No |
| FF | 100.0 | 58.3 | 84.3 | No |
| FF | 99.8 | 59.5 | 91.9 | No |

### Example 6. Corrugated Samples of 3-ply Paper Sheets

An antique desk-top hand cranked corrugator was purchased. The corrugator indicated U.S. Reexam Patent No. RE009,127 "Fluting-Machine", re-issued March 23rd, 1880 to H. Albrecht.

A sheet of TL1 was hung from inside an inverted 5-gallon pail and held over a boiling tea kettle to steam the sheet. The cast iron hand-cranked corrugator was warmed with a hair dryer, and the warm steamed sheet was promptly rippled. This was promptly bonded between two non-corrugated sheets of TL1 to make a rudimentary corrugated structure.
Single ply filled sheets were hand pressed in the lab and dried:

| Sheet Composition ID | EJ | EK |
|---|---|---|
| Water / g | 800 | 800 |
| Pulp / g | 4.5 | 4.5 |
| Flaked Perlite LD1006 / g | 9.0 | |
| iM30K glass bubbles / g | | 9.0 |
| Household ammonia / g | | 2 - 4 |

A sheet of EJ was hung from inside an inverted 5-gallon pail and held over a boiling tea kettle to steam the sheet. The cast iron hand-cranked corrugator was warmed with a hair dryer, and the warm steamed sheet was promptly fluted. This was promptly bonded between two non-corrugated sheets of EJ to make a rudimentary corrugated structure. This procedure was repeated using EK sheets for all three layers.

A sheet of TL1, EJ, and EK were each coated with Kaolin clay formulation 127-01, then dried, and then coated with 137-02 (BiLite (BASF) - bismuth oxychloride coated mica flakes) and dried. More uncoated sheets were steamed and fluted, and similar corrugated structures were produced incorporating one of the coated sheets with the coating side facing out as depicted in FIG. **20****.**

10 cm diameter disks were cut of each sample, and mounted into a cooler window for thermal testing. Prior to sealing with marine adhesive, the samples were gently pushed into the front of the cooler window so that the face of the composite was flush with the front of the cooler. 10cm discs of the following were also cut as controls: Aluminized bubble wrap, corrugated C-flute (35lbs.MSQ kraft liners with 23lb medium, Corrugated Supplies Inc.), corrugated B-flute (35lbs.MSQ kraft liners with 23lb medium, Corrugated Supplies Inc.), triple wall corrugated B-C flute (35lbs.MSQ kraft liners with 23lb medium, Corrugated Supplies Inc.)

Because these samples had significant thickness, temperature rise was monitored over an initial period of time until three consecutive 15-minute temperature readings showed an increase in temperature within +/- 0.1°C of each other. Upon attaining consistent temperature increase readings over 15 minutes, this was designated as pseudo-steady state. The temperature of the outside lamp-facing surface was also measured using a hand-held pyrometric infra-red thermometer, taking care to try not to allow reflections of the hot lamp from interfering. Usually, a pseudo-steady state situation of incremental temperature increases was established within 15 minutes of run time.

### Results of Controls

| Paper | corrugate | corrugate | Corrugate | Bubblewrap |
|---|---|---|---|---|
| | C-Flute | B-Flute | BC Flute | Aluminized |
| Ave. Thickness / mm | 4 | 3.175 | 6.35 | 3.175 |
| Coating 1 | - | - | - | - |
| Coating 2 (lamp facing) | - | - | - | - |
| 1hr Water T Rise / °C | 3.04 | 3.2 | 2.8 | 1.4 |
| Ave temp difference outer face of window vs. water / °C | 96.4 | 91.1 | 133.8 | Very noisy data. 74 +/- 25°C |
| W.m⁻² | 203 | 214 | 187 | 94 |

| Paper | corrugate | corrugate | corrugate | corrugate | corrugate | corrugate |
|---|---|---|---|---|---|---|
| | Control | Flake Perl. | Gls Bubls | Coated | Flk Perl. | Gls Bubls |
| | TL1 | EJ | EK | TL1 | EJ | EK |
| Av. Thkns / mm | 3.87 | 5.51 | 5.68 | 4.11 | 5.44 | 6.36 |
| Coating 1 | - | - | - | 127-01 | 127-01 | 127-01 |
| Coat. 2 (lamp) | - | - | - | 137-02 | 137-02 | 137-02 |
| 1hr T Rise / °C | 2.4 | 2.13 | NT* | 2 | 1.73 | 1.8 |
| Av. Delta T outer face of window vs. water / °C | 78.5 | 87.1 | NT* | 74.2 | 86.2 | 77.5 |
| W.m⁻² | 154 | 143 | | 134 | 116 | 120 |

| | | | | | | |
|---|---|---|---|---|---|---|
| * Structure failed during testing - delaminated. | | | | | | |

These data demonstrate the additive combination of addressing both radiative heat transfer as well as conductive heat transfer.

### Example 7:

### JL3-113-02 - Clay:

| | |
|---|---|
| 543g | Municipal Water |
| 66.9g | Tego Dispers 752W (Evonik) |
| 221.4g | Rovene 6400 (Mallard Creek Polymers) |
| 669g | Hydrite SB60 kaolin clay (Imerys) |
| Stir to disperse. | Shake vigorously immediately prior to use |

### JL3-118-01 - Thermal Top Coat

| | |
|---|---|
| 202g | Municipal Water |
| 7.89g | Tego Dispers 752W (Evonik) |
| 15g | Rovene 4100 (Mallard Creek Polymers) |
| 74g | BiLite 20 (BiOCI coated mica pigment) (BASF) |

Stir to disperse. Shake vigorously immediately prior to use.

Approximately 20 square feet of 40 lbs per 3,000 square feet kraft paper was hung vertically and coated with clay formulation JL3-113-02 using a 32 psi compressed air atomized high-pressure low volume paint spray gun, from about a 6" distance. The coating was applied in multiple passes until a uniform white layer was formed. A similar technique was used to overcoat a thin layer of JL3-118-01 coating, containing bismuth oxychloride-coated mica and a binder system. The paper was dried using a hair dryer, and allowed to equilibrate overnight. An average of 17 dried cut samples of coated and uncoated paper were weighed to determine a total coat weight of 80.8 g / m².

The paper had improved pigment rub-off compared to earlier formulations using similar materials, presumably, although without wishing to be bound by theory, because the binder concentration was increased and the surfactant package was changed. Interestingly, when the paper was folded or pleated, it made very little noise compared to the uncoated paper. Furthermore, the paper was found to be repulpable when tested.

It was noted that coated paper had a much smoother hand-feel than the uncoated paper. Haptic experiences can be difficult to describe, however, the paper felt more like handling a smooth fabric such as a microfiber polyester knit vs. kraft paper. The paper felt smoother, almost softer, and it made less noise when being handled compared to the uncoated paper. Furthermore, the paper was able to be folded without the coating flaking off. The paper was pleated to form pleats at approximately 1" intervals, with the intention for it to be used as insulating packaging.

## Claims

1. A repulpable insulated paper product comprising:
one or more paper layers; and
a smooth, heat-reflecting, thermally insulating coating on at least one outer surface of said one or more paper layers, said smooth, heat-reflecting, thermally insulating coating (a) comprising (i) from about 50.0 weight percent (wt%) to about 99.9 wt% of one or more insulating materials comprising bismuth oxychloride, mica, bismuth oxychloride-coated mica, zinc oxide, aluminum-doped zinc oxide, zinc sulfide, cadmium sulfide, bismuth vanadate, gypsum, sericite, powdered silicon, silver-coated glass bubbles, aluminum oxide, hollow polymeric microsphere pigments, or any mixture or combination thereof, and (ii) from about 50.0 wt% to about 0.1 wt% of a binder comprising (A) a latex binder selected from polymers synthesized using emulsion polymerization including poly(vinyl acetate), poly(acrylonitrile), poly(acrylates), poly(methacrylates), poly(butadiene), poly(styrene), poly(acrylic acid), and various copolymers of these polymers; or (B) a latex binder comprising a polymer or co-polymer of one or more monomers selected from styrene, butadiene, acrylic acid, acrylate, methacrylate, and vinyl acetate; (b) forms a continuous coating that completely covers the at least one outer surface; (c) reflects heat; and (d) reduces transfer of heat through the repulpable insulated paper product,
wherein the repulpable integral paper product is repulpable as determined by the "Voluntary Standard for Repulping and Recycling Corrugated Fiberboard treated to Improve Its Performance in the Presence of Water and Water Vapor Protocol of 2013" with 85% or more of recovered fibers from the repulped integral paper product being accepted, not rejected, using this test.

2. The repulpable insulated paper product of claim 1, wherein the one or more paper layers comprises a single paper layer.

3. The repulpable insulated paper product of claim 1, wherein the one or more paper layers comprises two or more paper layers.

4. The repulpable insulated paper product of any one of claims 1 to 3, wherein the smooth, heat-reflecting, thermally insulating coating comprises one or more insulating materials comprising bismuth oxychloride, mica, zinc oxide, bismuth oxychloride-coated mica, or any mixture or combination thereof.

5. The repulpable insulated paper product of any one of claims 1 to 4, wherein the smooth, heat-reflecting, thermally insulating coating comprises two or more coating layers with each coating layer comprising said insulating material and said binder.

6. The repulpable insulated paper product of claim 5, wherein said two or more coating layers comprise (i) a first coating applied onto the one or more paper layers and comprising zinc oxide, aluminum-doped zinc oxide, or any mixture or combination thereof, and (ii) a second coating applied onto the first coating and comprising bismuth oxychloride, bismuth oxychloride-coated mica, or any mixture or combination thereof.

7. The repulpable insulated paper product of any one of claims 1 to 6, further comprising a treatment to impart water or grease resistance to the repulpable insulated paper product, wherein the treatment comprises (i) adding one or more treatment additives to one or more of the one or more paper layers, or (ii) adding one or more treatment additives to the smooth, heat-reflecting, thermally insulating coating, or (iii) adding a water or grease resistance layer comprising one or more treatment additives onto the repulpable insulated paper product, or any combination of (i) to (iii), and wherein the one or more treatment additives comprise a wax emulsion, a latex binder, a styrene acrylic based copolymer emulsion, a styrene acrylic copolymer emulsion binder, a poly(vinylidene chloride) (PVDC) latex, a blend including a styrene acrylic copolymer emulsion, a poly(ethylene) wax and clay, a poly(vinylidene chloride) (PVDC) latex, or any combination thereof.

8. The repulpable insulated paper product of any one of claims 1 to 7, wherein the repulpable insulated paper product comprises a void-containing repulpable insulated paper product, and wherein the void-containing repulpable insulated paper product comprises a corrugated paper product.

9. The repulpable insulated paper product of any one of claims 1 and 3 to 8, wherein the repulpable integral paper product comprises (i) a first linerboard layer comprising one or more first paper layers, (ii) a second linerboard layer comprising one or more second paper layers, and (iii) (a) a fluted paper layer comprising one or more fluted paper layers or (b) a honeycomb layer positioned between the first linerboard layer and the second linerboard layer, and (I) each of (i) said first linerboard layer, (ii) said second linerboard layer, and (iii) (a) said fluted paper layer or (b) said honeycomb layer may independently comprise insulating material therein or thereon, and (II) said smooth, heat-reflecting, thermally insulating coating is present on (i) an outer surface of said first linerboard layer, (ii) an outer surface of said second linerboard layer, or (iii) both (i) and (ii).

10. The repulpable insulated paper product of claim 9, wherein each of (i) said first linerboard layer, (ii) said second linerboard layer, and (iii) (a) said fluted paper layer or (b) said honeycomb layer independently comprises the repulpable insulated paper product of any one of claims 1 to 9.

11. The repulpable insulated paper product of any one of claims 1 to 10, wherein the repulpable insulated paper product further comprises one or more additional non-paper layers, wherein the one or more additional non-paper layers comprise a clay-containing layer, a coating that provides a lower or higher emissivity of the repulpable insulated paper product, a pigment-containing layer, or any combination thereof.

12. The repulpable insulated paper product of any one of claims 1 to 11, wherein the repulpable insulated paper product comprises (i) a first coating applied onto an outer surface of the one or more paper layers, said first coating comprising kaolin clay; and (ii) said smooth, heat-reflecting, thermally insulating coating on the first coating.

13. The repulpable insulated paper product of any one of claims 1 to 12, wherein the repulpable insulated paper product is molded to form a three-dimensional object (e.g., a cup or container).

14. A repulpable storage container comprising the repulpable insulated paper product of any one of claims 1 to 13, wherein the repulpable storage container comprises a storage volume at least partially surrounded by one or more container walls, and wherein the storage container comprises an insulating wrapper for a food item, a cup, a mug, a flask, a thermos, a clam shell type box packaging for hot food, a salad container for chilled food, a padded envelope, a shipping container, or a cup sleeve.

15. A method of using the repulpable insulated paper product of any one of claims 1 to 13 or the repulpable storage container of claim 14, said method comprising:
insulating an object via the repulpable insulated paper product or the repulpable storage container, wherein the object is a food item, a medicine, or any other item that is desirably kept at a cool temperature (e.g., a temperature below room temperature or a refrigerating temperature) or at an elevated temperature (e.g., a temperature above room temperature or a hot-out-of-the-oven temperature).

## Patentansprüche

1. Repulpierbares isoliertes Papierprodukt, umfassend:
eine oder mehrere Papierschichten; und
eine glatte, wärmereflektierende, thermisch isolierende Beschichtung auf mindestens einer Außenfläche der einen oder mehreren Papierschichten, wobei die glatte, wärmereflektierende, thermisch isolierende Beschichtung (a) (i) von etwa 50,0 Gewichtsprozent (Gew.-%) bis etwa 99,9 Gew.-% eines oder mehrere Isoliermaterialien umfasst, umfassend Bismutoxychlorid, Glimmer, mit Bismutoxychlorid beschichtetem Glimmer, Zinkoxid, Aluminium-dotiertem Zinkoxid, Zinksulfid, Cadmiumsulfid, Bismutvanadat, Gips, Serizit, pulverförmigem Silizium, silberbeschichteten Glasbläschen, Aluminiumoxid,
hohlen polymeren Mikrosphärenpigmenten oder einer beliebigen Mischung oder
Kombination davon, und (ii) von etwa 50,0 Gew.-% bis etwa 0,1 Gew.-% eines Bindemittels umfasst, umfassend (A) ein Latexbindemittel, ausgewählt aus Polymeren, die unter Verwendung von Emulsionspolymerisation synthetisiert wurden, umfassend Poly(vinylacetat), Poly(acrylnitril), Poly(acrylate), Poly(methacrylate), Poly(butadien), Poly(styrol), Poly(acrylsäure) und verschiedene Copolymere dieser Polymere; oder (B) ein Latexbindemittel, umfassend ein Polymer oder Copolymer aus einem oder mehreren Monomeren, ausgewählt aus Styrol, Butadien, Acrylsäure, Acrylat, Methacrylat und
Vinylacetat ausgewählt sind; (b) eine kontinuierliche Beschichtung bildet, die die mindestens eine Außenfläche vollständig bedeckt; (c) Wärme reflektiert; und (d) die Übertragung von Wärme durch das repulpierbare isolierte Papierprodukt reduziert,
wobei das repulpierbare integrale Papierprodukt repulpierbar ist, wie durch den "Voluntary Standard for Repulping and Recycling Corrugated Fiberboard treated to Improve Its Performance in the Presence of Water and Water Vapor Protocol of 2013" festgelegt, wobei 85 % oder mehr der rückgewonnenen Fasern von dem repulpierbaren integralen Papierprodukt unter Verwendung dieses Tests akzeptiert und nicht zurückgewiesen werden.

2. Repulpierbares isoliertes Papierprodukt nach Anspruch 1, wobei die eine oder mehreren Papierschichten eine einzelne Papierschicht umfassen.

3. Repulpierbares isoliertes Papierprodukt nach Anspruch 1, wobei die eine oder mehreren Papierschichten zwei oder mehr Papierschichten umfassen.

4. Repulpierbares isoliertes Papierprodukt nach einem der Ansprüche 1 bis 3, wobei die glatte, wärmereflektierende, thermisch isolierende Beschichtung ein oder mehrere Isoliermaterialien umfasst, umfassend Bismutoxychlorid, Glimmer, Zinkoxid, mit Bismutoxychlorid beschichtetem Glimmer oder eine beliebige Mischung oder Kombination davon.

5. Repulpierbares isoliertes Papierprodukt nach einem der Ansprüche 1 bis 4, wobei die glatte, wärmereflektierende, thermisch isolierende Beschichtung zwei oder mehr Beschichtungsschichten umfasst, wobei jede Beschichtungsschicht das Isoliermaterial und das Bindemittel umfasst.

6. Repulpierbares isoliertes Papierprodukt nach Anspruch 5, wobei die zwei oder mehr Beschichtungsschichten (i) eine erste Beschichtung umfasst, die auf die eine oder mehreren Papierschichten aufgetragen ist und Zinkoxid, Aluminium-dotiertes Zinkoxid oder eine beliebige Mischung oder Kombination davon umfasst, und (ii) eine zweite Beschichtung umfasst, die auf die erste Beschichtung aufgetragen ist und Bismutoxychlorid, mit Bismutoxychlorid beschichtetem Glimmer oder eine beliebige Mischung oder Kombination davon umfasst.

7. Repulpierbares isoliertes Papierprodukt nach einem der Ansprüche 1 bis 6, ferner umfassend eine Behandlung, um dem repulpierbaren isolierten Papierprodukt Wasser- oder Fettresistenz zu verleihen, wobei die Behandlung (i) Zugeben eines oder mehrerer Behandlungsadditive zu einer oder mehreren der einen oder mehreren Papierschichten oder (ii) Zugeben eines oder mehrerer Behandlungsadditive zu der glatten, wärmereflektierenden, thermisch isolierenden Beschichtung oder (iii) Auftragen einer wasser- oder fettresistente Schicht, umfassend ein oder mehrere Behandlungsadditive, auf das repulpierbare isolierte Papierprodukt oder eine beliebige Kombination von (i) bis (iii) umfasst, und wobei das eine oder die mehreren Behandlungsadditive eine Wachsemulsion, ein Latexbindemittel, eine Copolymer-Emulsion auf Styrol-Acryl-Basis, ein Styrol-Acryl-Copolymer-Emulsionsbindemittel, ein Poly(vinylidenchlorid) (PVDC)-Latex, eine Mischung, umfassend eine Styrol-Acryl-Copolymer-Emulsion, ein Poly(ethylen)wachs und Ton, ein Poly(vinylidenchlorid) (PVDC)-Latex, oder eine beliebige Kombination davon umfasst.

8. Repulpierbares isoliertes Papierprodukt nach einem der Ansprüche 1 bis 7, wobei das repulpierbare isolierte Papierprodukt ein Hohlräume enthaltendes repulpierbares isoliertes Papierprodukt umfasst und wobei das Hohlräume enthaltende repulpierbare isolierte Papierprodukt ein gewelltes Papierprodukt umfasst.

9. Repulpierbares isoliertes Papierprodukt nach einem der Ansprüche 1 und 3 bis 8, wobei das repulpierbare integrale Papierprodukt (i) eine erste Deckenpapier-Schicht, umfassend eine oder mehrere erste Papierschichten, (ii) eine zweite Deckenpapier-Schicht, umfassend eine oder mehrere zweite Papierschichten, und (iii) (a) eine geriffelte Papierschicht, umfassend eine oder mehrere geriffelte Papierschichten, umfasst, oder (b) eine Wabenschicht, die zwischen der ersten Deckenpapier-Schicht und der zweiten Deckenpapier-Schicht angeordnet ist, umfasst, und (I) jede von (i) der ersten Deckenpapier-Schicht, (ii) der zweiten Deckenpapier-Schicht und (iii) (a) der geriffelten Papierschicht oder (b) der Wabenschicht unabhängig voneinander Isoliermaterial darin oder darauf umfassen kann, und (II) die glatte, wärmereflektierende, thermisch isolierende Beschichtung auf (i) einer Außenfläche der ersten Deckenpapier-Schicht, (ii) einer Außenfläche der zweiten Deckenpapier-Schicht oder (iii) sowohl (i) als auch (ii) vorhanden ist.

10. Repulpierbares isoliertes Papierprodukt nach Anspruch 9, wobei jede (i) der ersten Deckenpapier-Schicht, (ii) der zweiten Deckenpapier-Schicht und (iii) (a) der geriffelten Papierschicht oder (b) der Wabenschicht unabhängig voneinander das repulpierbare isolierte Papierprodukt nach einem der Ansprüche 1 bis 9 umfasst.

11. Repulpierbares isoliertes Papierprodukt nach einem der Ansprüche 1 bis 10, wobei das repulpierbare isolierte Papierprodukt ferner eine oder mehrere zusätzliche Nicht-Papierschichten umfasst, wobei die eine oder mehreren zusätzlichen Nicht-Papierschichten eine tonhaltige Schicht, eine Beschichtung, die ein geringeres oder höheres Emissionsvermögen des repulpierbaren isolierten Papierprodukts bewirkt, eine pigmenthaltige Schicht oder eine beliebige Kombination davon umfassen.

12. Repulpierbares isoliertes Papierprodukt nach einem der Ansprüche 1 bis 11, wobei das repulpierbare isolierte Papierprodukt (i) eine erste Beschichtung, die auf eine Außenfläche der einen oder mehreren Papierschichten aufgebracht ist, wobei die erste Beschichtung Kaolinton umfasst; und (ii) die glatte, wärmereflektierende, thermisch isolierende Beschichtung auf der ersten Beschichtung umfasst.

13. Repulpierbares isoliertes Papierprodukt nach einem der Ansprüche 1 bis 12, wobei das repulpierbare isolierte Papierprodukt geformt ist, um ein dreidimensionales Objekt (z. B. einen Becher oder Behälter) zu bilden.

14. Repulpierbarer Lagerbehälter, umfassend das repulpierbare isolierte Papierprodukt nach einem der Ansprüche 1 bis 13, wobei der repulpierbare Lagerbehälter ein Lagervolumen umfasst, das zumindest teilweise von einer oder mehreren Behälterwänden umgeben ist, und wobei der Lagerbehälter eine isolierende Hülle für ein Lebensmittel, einen Becher, einen Krug, eine Flasche, eine Thermoskanne, eine Box-Verpackung vom Clam-Shell-Typ für heiße Lebensmittel, einen Salatbehälter für gekühlte Lebensmittel, einen gepolsterten Umschlag, einen Versandbehälter oder eine Becherhülle umfasst.

15. Verfahren zum Verwenden des repulpierbaren isolierten Papierprodukts nach einem der Ansprüche 1 bis 13 oder des repulpierbaren Lagerbehälters nach Anspruch 14, wobei das Verfahren umfasst:
Isolieren eines Objekts mittels des repulpierbaren isolierten Papierprodukts oder des repulpierbaren Lagerbehälters, wobei das Objekt ein Lebensmittel, ein Medikament oder ein beliebiger anderer Gegenstand ist, das vorzugsweise bei einer kühlen Temperatur (z. B.
einer Temperatur unterhalb der Raumtemperatur oder einer Kühltemperatur) oder bei einer erhöhten Temperatur (z. B. einer Temperatur oberhalb der Raumtemperatur oder einer Temperatur wie direkt aus dem Ofen) gehalten wird.

## Revendications

1. Produit en papier isolant repulpable comprenant :
une ou plusieurs couches de papier ; et
un revêtement lisse, réfléchissant la chaleur et thermiquement isolant sur au moins une surface extérieure de ladite ou desdites couches de papier, ledit revêtement lisse, réfléchissant la chaleur et thermiquement isolant (a) comprenant (i) d'environ 50,0 % en poids (wt%) à environ 99. 9 % en poids d'un ou plusieurs matériaux isolants comprenant de l'oxychlorure de bismuth, du mica, du mica recouvert d'oxychlorure de bismuth, de l'oxyde de zinc, de l'oxyde de zinc dopé à l'aluminium, du sulfure de zinc, du sulfure de cadmium, du vanadate de bismuth, du gypse, de la séricite, de la poudre de silicium, des bulles de verre recouvertes d'argent, de l'oxyde d'aluminium, des pigments de microsphères polymères creuses, ou tout mélange ou combinaison de ceux-ci, et (ii) d'environ 50,0 % en poids à environ 0,1 % en poids d'un liant comprenant (A) un liant en latex choisi parmi les polymères synthétisés par polymérisation en émulsion, y compris le poly(acétate de vinyle), le poly(acrylonitrile), les poly(acrylates), les poly(méthacrylates), le poly(butadiène), le poly(styrène), l'acide poly(acrylique), et divers copolymères de ces polymères ; ou (B) un liant en latex comprenant un polymère ou un copolymère d'un ou de plusieurs monomères choisis parmi le styrène, le butadiène, l'acide acrylique, l'acrylate, le méthacrylate et l'acétate de vinyle ; (b) forme un revêtement continu qui recouvre complètement au moins une surface extérieure ; (c) réfléchit la chaleur ; et (d) réduit le transfert de chaleur à travers le produit en papier isolant repulpable,
dans lequel le produit en papier intégral repulpable est repulpable conformément à la « norme volontaire du protocole de 2013 pour le repulpage et le recyclage du carton ondulé traité pour améliorer sa performance en présence d'eau et de vapeur d'eau », dont 85 % ou plus des fibres récupérées du produit en papier intégral repulpé étant sont acceptées, et non rejetées, à l'aide de ce test.

2. Le produit en papier isolant repulpable de la revendication 1, dans lequel la ou les couches de papier comprennent une seule couche de papier.

3. Produit en papier isolant repulpable de la revendication 1, dans lequel la ou les couches de papier comprennent deux ou plusieurs couches de papier.

4. Le produit en papier isolant repulpable de l'une des revendications 1 à 3, dans lequel le revêtement lisse, réfléchissant la chaleur et thermiquement isolant comprend un ou plusieurs matériaux isolants comprenant de l'oxychlorure de bismuth, du mica, de l'oxyde de zinc, du mica recouvert d'oxychlorure de bismuth, ou tout mélange ou combinaison de ceux-ci.

5. Le produit en papier isolant repulpable de l'une des revendications 1 à 4, dans lequel le revêtement lisse, réfléchissant la chaleur et thermiquement isolant comprend deux couches de revêtement ou plus, chaque couche de revêtement comprenant ledit matériau isolant et ledit liant.

6. Le produit en papier isolant repulpable de la revendication 5, dans lequel ces deux couches de revêtement ou plus comprennent (i) un premier revêtement appliqué sur la ou les couches de papier et comprenant de l'oxyde de zinc, de l'oxyde de zinc dopé à l'aluminium, ou tout mélange ou combinaison de ceux-ci, et (ii) un second revêtement appliqué sur le premier revêtement et comprenant de l'oxychlorure de bismuth, du mica recouvert d'oxychlorure de bismuth, ou tout mélange ou combinaison de ceux-ci.

7. Le produit en papier isolant repulpable de l'une des revendications 1 à 6, comprenant en outre un traitement pour conférer une résistance à l'eau ou à la graisse au produit en papier isolant repulpable, dans lequel le traitement comprend (i) l'ajout d'un ou plusieurs additifs de traitement à une ou plusieurs des couches de papier, ou (ii) l'ajout d'un ou plusieurs additifs de traitement au revêtement lisse, réfléchissant la chaleur et thermiquement isolant, ou (iii) l'ajout d'une couche de résistance à l'eau ou à la graisse comprenant un ou plusieurs additifs de traitement sur le produit en papier isolant repulpable, ou toute combinaison de (i) à (iii), et dans laquelle le ou les additifs de traitement comprennent une émulsion de cire, un liant en latex, une émulsion de copolymère à base de styrène acrylique, un liant d'émulsion de copolymère de styrène acrylique, un latex de poly(chlorure de vinylidène) (PVDC), un mélange comprenant une émulsion de copolymère de styrène acrylique, une cire de poly(éthylène) et de l'argile, un latex de poly(chlorure de vinylidène) (PVDC), ou toute combinaison de ceux-ci.

8. Le produit en papier isolant repulpable de l'une des revendications 1 à 7, dans lequel le produit en papier isolant repulpable comprend un produit en papier isolant repulpable contenant du vide, et dans lequel le produit en papier isolant repulpable contenant du vide comprend un produit en papier ondulé.

9. Le produit en papier isolant repulpable de l'une des revendications 1 et 3 à 8, dans lequel le produit en papier intégral repulpable comprend (i) une première couche de carton comprenant une ou plusieurs premières couches de papier, (ii) une seconde couche de carton comprenant une ou plusieurs secondes couches de papier, et (iii) (a) une couche de papier cannelé comprenant une ou plusieurs couches de papier cannelé ou (b) une couche en nid d'abeilles positionnée entre la première couche de carton et la seconde couche de carton, et (l) chacune (i) de ladite première couche de carton, (ii) de ladite seconde couche de carton, et (iii) (a) de ladite couche de papier cannelé ou (b) de ladite couche en nid d'abeilles peut comprendre indépendamment un matériau isolant dans ou sur elle, et (II) ledit revêtement lisse, réfléchissant la chaleur, thermiquement isolant est présent sur (i) une surface extérieure de ladite première couche de carton, (ii) une surface extérieure de ladite seconde couche de carton, ou (iii) à la fois (i) et (ii).

10. Produit en papier isolant repulpable de la revendication 9, dans lequel chacun (i) de ladite première couche de carton, (ii) de ladite seconde couche de carton, et (iii) (a) de ladite couche de papier cannelé ou (b) de ladite couche en nid d'abeilles comprend indépendamment le produit en papier isolant repulpable de l'une quelconque des revendications 1 à 9.

11. Le produit en papier isolant repulpable de l'une des revendications 1 à 10, dans lequel le produit en papier isolant repulpable comprend en outre une ou plusieurs couches supplémentaires non papier, dans lesquelles la ou les couches supplémentaires non papier comprennent une couche contenant de l'argile, un revêtement qui réduit ou augmente l'émissivité du produit en papier isolant repulpable, une couche contenant des pigments, ou toute combinaison de ceux-ci.

12. Le produit en papier isolant repulpable de l'une des revendications 1 à 11, dans lequel le produit en papier isolant repulpable comprend (i) un premier revêtement appliqué sur une surface extérieure d'une ou plusieurs couches de papier, ledit premier revêtement comprenant de l'argile kaolinique ; et (ii) ledit revêtement lisse, réfléchissant la chaleur et thermiquement isolant sur le premier revêtement.

13. Le produit en papier isolant repulpable de l'une des revendications 1 à 12, dans lequel le produit en papier isolant repulpable est moulé pour former un objet tridimensionnel (par exemple, une tasse ou un récipient).

14. Récipient de stockage repulpable comprenant le produit en papier isolant repulpable de l'une des revendications 1 à 13, dans lequel le récipient de stockage repulpable comprend un volume de stockage au moins partiellement entouré par une ou plusieurs parois du récipient, et dans lequel le récipient de stockage comprend un emballage isolant pour un produit alimentaire, une tasse, un mug, une gourde, un thermos, une boîte d' emballage à clapets pour des aliments chauds, un récipient à salade pour des aliments réfrigérés, une enveloppe matelassée, un récipient d'expédition, ou un manchon de tasse.

15. Méthode d'utilisation du produit en papier isolant repulpable de l'une des revendications 1 à 13 ou du récipient de stockage repulpable de la revendication 14, ladite méthode comprenant :
l'isolation d'un objet par le produit en papier isolant repulpable ou le récipient de stockage repulpable, dans laquelle l'objet est un aliment, un médicament ou tout autre article qu'il est souhaitable de conserver à une température fraîche (par exemple, une température inférieure à la température ambiante ou une température de réfrigération) ou à une température élevée (par exemple, une température supérieure à la température ambiante ou une température de sortie du four).
